



US011147346B2

(12) **United States Patent**  
**Takani**

(10) **Patent No.:** **US 11,147,346 B2**  
(45) **Date of Patent:** **Oct. 19, 2021**

(54) **TAPE FOR SLIDE FASTENER**

(71) Applicant: **YKK Corporation**, Tokyo (JP)

(72) Inventor: **Go Takani**, Guangdong (CN)

(73) Assignee: **YKK Corporation**, Tokyo (JP)

(\*) Notice: Subject to any disclaimer, the term of this patent is extended or adjusted under 35 U.S.C. 154(b) by 125 days.

(21) Appl. No.: **16/203,525**

(22) Filed: **Nov. 28, 2018**

(65) **Prior Publication Data**

US 2019/0166959 A1 Jun. 6, 2019

(30) **Foreign Application Priority Data**

Dec. 1, 2017 (CN) ..... 201711249063.0  
Dec. 1, 2017 (CN) ..... 201721651179.2

(51) **Int. Cl.**

*A44B 19/34* (2006.01)  
*A44B 19/12* (2006.01)

(52) **U.S. Cl.**

CPC ..... *A44B 19/34* (2013.01); *A44B 19/12* (2013.01); *A44B 19/346* (2013.01)

(58) **Field of Classification Search**

CPC ..... A44B 19/34; A44B 19/12; A44B 19/346;  
A44B 19/343; Y10T 24/252

See application file for complete search history.

(56) **References Cited**

U.S. PATENT DOCUMENTS

4,149,569 A \* 4/1979 Frohlich ..... A44B 19/12  
139/11  
5,699,592 A \* 12/1997 Shimono ..... A44B 19/12  
24/432

7,152,438 B2 \* 12/2006 Matsuda ..... A44B 19/343  
66/192

9,169,583 B2 \* 10/2015 Hasegawa ..... A44B 19/346  
9,668,549 B2 \* 6/2017 Tsuzuyama ..... D03D 1/00

2005/0235466 A1 \* 10/2005 Segawa ..... A44B 19/34  
24/396

2011/0033687 A1 2/2011 Deguchi  
(Continued)

FOREIGN PATENT DOCUMENTS

CN 103124505 A 5/2013  
GB 1450162 A 9/1976  
(Continued)

OTHER PUBLICATIONS

Office Action, Japanese Patent Application No. 2018-208264, dated Oct. 23, 2019.

*Primary Examiner* — Robert Sandy

*Assistant Examiner* — Louis A Mercado

(74) *Attorney, Agent, or Firm* — Kilpatrick Townsend & Stockton LLP

(57) **ABSTRACT**

A tape for a slide fastener includes warps and wefts. A yarn count of warps among yarns forming the fastener tape is set to 22-28 dTex. A weave density of the warps is set to 205-231 yarns/inch. A yarn count of wefts among the yarns forming the fastener tape is set to 81-87 dTex. A weave density of the wefts is set to 42-48 yarns/inch. The weft is a multifilament formed by bundling 33-39 monofilaments. According to one embodiment, the yarn count of the warps is set to 25 dTex, the weave density of the warps is set to 210-226 yarns/inch, the yarn count of the weft is set to 84 dTex, the weave density of the wefts is set to 43-46 yarns/inch, and the weft is a multifilament formed by bundling 36 monofilaments.

**1 Claim, 83 Drawing Sheets**



(56)

**References Cited**

U.S. PATENT DOCUMENTS

2013/0177734 A1 7/2013 Hasegawa et al.  
2019/0166959 A1\* 6/2019 Takani ..... A44B 19/34

FOREIGN PATENT DOCUMENTS

|    |                |         |
|----|----------------|---------|
| JP | S54-145306 A   | 3/1953  |
| JP | S49-043745 A   | 4/1974  |
| JP | 2006-175129 A  | 7/2006  |
| JP | 2013-177731 A  | 9/2013  |
| JP | 2014-214388 A  | 11/2014 |
| WO | 2014/013616 A1 | 1/2014  |

\* cited by examiner

FIG. 1



FIG. 2



FIG. 3



FIG. 4



## FIG. 5

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2500                            | 20.8225                      |  | 2500                            | 23.7313                      |
| 2499                            | 20.6391                      |  | 2499                            | 23.9299                      |
| 2498                            | 21.4634                      |  | 2498                            | 24.1843                      |
| 2497                            | 19.9055                      |  | 2497                            | 23.1784                      |
| 2496                            | 20.9035                      |  | 2496                            | 22.7633                      |
| 2495                            | 20.7094                      |  | 2495                            | 23.4852                      |
| 2494                            | 20.7466                      |  | 2494                            | 24.4853                      |
| 2493                            | 21.6674                      |  | 2493                            | 24.5625                      |
| 2492                            | 19.7379                      |  | 2492                            | 24.057                       |
| 2491                            | 19.9436                      |  | 2491                            | 23.0936                      |
| 2490                            | 19.834                       |  | 2490                            | 22.3935                      |
| 2489                            | 19.5324                      |  | 2489                            | 22.4975                      |
| 2488                            | 20.264                       |  | 2488                            | 22.4186                      |
| 2487                            | 19.8651                      |  | 2487                            | 21.9792                      |
| 2486                            | 19.8963                      |  | 2486                            | 21.8949                      |
| 2485                            | 20.4442                      |  | 2485                            | 22.1385                      |
| 2484                            | 21.7887                      |  | 2484                            | 23.1309                      |
| 2483                            | 22.4228                      |  | 2483                            | 23.553                       |
| 2482                            | 21.6515                      |  | 2482                            | 23.2246                      |
| 2481                            | 21.1329                      |  | 2481                            | 22.9994                      |
| 2480                            | 20.2581                      |  | 2480                            | 22.2106                      |
| 2479                            | 20.2413                      |  | 2479                            | 22.1436                      |
| 2478                            | 19.5081                      |  | 2478                            | 21.5618                      |
| 2477                            | 19.6998                      |  | 2477                            | 21.7823                      |
| 2476                            | 19.3997                      |  | 2476                            | 22.4206                      |
| 2475                            | 19.7047                      |  | 2475                            | 23.3312                      |
| 2474                            | 21.8455                      |  | 2474                            | 24.9918                      |
| 2473                            | 21.3373                      |  | 2473                            | 24.5923                      |

## FIG. 6

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2472                            | 22.1188                      |  | 2472                            | 24.9023                      |
| 2471                            | 22.4501                      |  | 2471                            | 25.8877                      |
| 2470                            | 20.8589                      |  | 2470                            | 24.3681                      |
| 2469                            | 22.2017                      |  | 2469                            | 25.3144                      |
| 2468                            | 22.4576                      |  | 2468                            | 25.0365                      |
| 2467                            | 21.1625                      |  | 2467                            | 22.7728                      |
| 2466                            | 20.931                       |  | 2466                            | 22.7941                      |
| 2465                            | 19.8976                      |  | 2465                            | 22.0328                      |
| 2464                            | 18.6494                      |  | 2464                            | 21.1559                      |
| 2463                            | 18.8941                      |  | 2463                            | 21.8044                      |
| 2462                            | 20.0029                      |  | 2462                            | 21.9526                      |
| 2461                            | 20.7885                      |  | 2461                            | 22.2146                      |
| 2460                            | 21.4467                      |  | 2460                            | 23.1074                      |
| 2459                            | 22.6943                      |  | 2459                            | 22.7293                      |
| 2458                            | 22.9098                      |  | 2458                            | 23.0387                      |
| 2457                            | 22.0748                      |  | 2457                            | 22.2233                      |
| 2456                            | 21.7534                      |  | 2456                            | 22.1873                      |
| 2455                            | 20.7829                      |  | 2455                            | 22.6151                      |
| 2454                            | 19.6583                      |  | 2454                            | 22.5766                      |
| 2453                            | 19.9917                      |  | 2453                            | 23.5267                      |
| 2452                            | 19.9811                      |  | 2452                            | 23.439                       |
| 2451                            | 19.5569                      |  | 2451                            | 23.1999                      |
| 2450                            | 20.3724                      |  | 2450                            | 23.8071                      |
| 2449                            | 20.0208                      |  | 2449                            | 24.0868                      |
| 2448                            | 19.28                        |  | 2448                            | 22.822                       |
| 2447                            | 19.9225                      |  | 2447                            | 23.0199                      |
| 2446                            | 20.83                        |  | 2446                            | 22.8693                      |
| 2445                            | 21.7515                      |  | 2445                            | 23.3889                      |

## FIG. 7

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2444                            | 23.1061                      |  | 2444                            | 25.2337                      |
| 2443                            | 22.9385                      |  | 2443                            | 25.7043                      |
| 2442                            | 21.8865                      |  | 2442                            | 25.05                        |
| 2441                            | 21.9247                      |  | 2441                            | 24.2426                      |
| 2440                            | 22.232                       |  | 2440                            | 24.274                       |
| 2439                            | 21.711                       |  | 2439                            | 23.9744                      |
| 2438                            | 20.9793                      |  | 2438                            | 24.2496                      |
| 2437                            | 20.6009                      |  | 2437                            | 23.7282                      |
| 2436                            | 19.7202                      |  | 2436                            | 23.4627                      |
| 2435                            | 20.294                       |  | 2435                            | 23.6767                      |
| 2434                            | 20.4654                      |  | 2434                            | 23.0543                      |
| 2433                            | 19.9449                      |  | 2433                            | 23.6159                      |
| 2432                            | 20.9733                      |  | 2432                            | 23.5008                      |
| 2431                            | 20.3513                      |  | 2431                            | 23.8083                      |
| 2430                            | 21.2849                      |  | 2430                            | 24.6358                      |
| 2429                            | 22.0859                      |  | 2429                            | 24.9119                      |
| 2428                            | 21.4754                      |  | 2428                            | 24.74                        |
| 2427                            | 21.3207                      |  | 2427                            | 23.4769                      |
| 2426                            | 20.6348                      |  | 2426                            | 23.3148                      |
| 2425                            | 19.9564                      |  | 2425                            | 22.7634                      |
| 2424                            | 19.8995                      |  | 2424                            | 23.1056                      |
| 2423                            | 19.848                       |  | 2423                            | 23.8198                      |
| 2422                            | 20.0402                      |  | 2422                            | 23.9697                      |
| 2421                            | 19.8612                      |  | 2421                            | 23.6663                      |
| 2420                            | 20.055                       |  | 2420                            | 23.7263                      |
| 2419                            | 20.5827                      |  | 2419                            | 23.5758                      |
| 2418                            | 20.5665                      |  | 2418                            | 24.5248                      |
| 2417                            | 20.7555                      |  | 2417                            | 24.6641                      |

## FIG. 8

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2416                            | 20.2189                      |  | 2416                            | 23.2915                      |
| 2415                            | 20.2727                      |  | 2415                            | 23.9537                      |
| 2414                            | 20.0417                      |  | 2414                            | 22.7539                      |
| 2413                            | 20.1488                      |  | 2413                            | 22.0552                      |
| 2412                            | 20.5083                      |  | 2412                            | 23.2017                      |
| 2411                            | 19.8625                      |  | 2411                            | 22.3862                      |
| 2410                            | 20.9973                      |  | 2410                            | 22.9291                      |
| 2409                            | 20.6671                      |  | 2409                            | 23.8525                      |
| 2408                            | 20.3759                      |  | 2408                            | 23.2581                      |
| 2407                            | 20.8696                      |  | 2407                            | 23.8264                      |
| 2406                            | 19.4243                      |  | 2406                            | 23.4334                      |
| 2405                            | 20.1488                      |  | 2405                            | 23.6688                      |
| 2404                            | 20.1377                      |  | 2404                            | 23.596                       |
| 2403                            | 20.0627                      |  | 2403                            | 22.9663                      |
| 2402                            | 20.4416                      |  | 2402                            | 22.7601                      |
| 2401                            | 19.5082                      |  | 2401                            | 22.6324                      |
| 2400                            | 20.0927                      |  | 2400                            | 23.0122                      |
| 2399                            | 19.9345                      |  | 2399                            | 23.2941                      |
| 2398                            | 20.3013                      |  | 2398                            | 23.4888                      |
| 2397                            | 20.7075                      |  | 2397                            | 23.342                       |
| 2396                            | 19.9206                      |  | 2396                            | 23.1581                      |
| 2395                            | 20.2521                      |  | 2395                            | 23.164                       |
| 2394                            | 19.9561                      |  | 2394                            | 23.2585                      |
| 2393                            | 20.087                       |  | 2393                            | 23.4739                      |
| 2392                            | 20.6726                      |  | 2392                            | 23.7404                      |
| 2391                            | 20.5748                      |  | 2391                            | 23.6499                      |
| 2390                            | 20.2693                      |  | 2390                            | 23.4812                      |
| 2389                            | 20.1671                      |  | 2389                            | 23.4296                      |

## FIG. 9

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2388                            | 19.4638                      |  | 2388                            | 23.4276                      |
| 2387                            | 19.3935                      |  | 2387                            | 23.3674                      |
| 2386                            | 19.0118                      |  | 2386                            | 23.0111                      |
| 2385                            | 18.5461                      |  | 2385                            | 22.8014                      |
| 2384                            | 19.0091                      |  | 2384                            | 23.2655                      |
| 2383                            | 18.8866                      |  | 2383                            | 22.924                       |
| 2382                            | 19.8576                      |  | 2382                            | 23.6499                      |
| 2381                            | 20.0959                      |  | 2381                            | 23.7151                      |
| 2380                            | 19.8294                      |  | 2380                            | 23.077                       |
| 2379                            | 20.1184                      |  | 2379                            | 23.8623                      |
| 2378                            | 19.7567                      |  | 2378                            | 23.2292                      |
| 2377                            | 19.9137                      |  | 2377                            | 22.8513                      |
| 2376                            | 19.6745                      |  | 2376                            | 22.6335                      |
| 2375                            | 20.009                       |  | 2375                            | 22.93                        |
| 2374                            | 20.249                       |  | 2374                            | 23.4342                      |
| 2373                            | 20.4103                      |  | 2373                            | 23.9757                      |
| 2372                            | 20.6855                      |  | 2372                            | 23.877                       |
| 2371                            | 20.369                       |  | 2371                            | 23.674                       |
| 2370                            | 20.0776                      |  | 2370                            | 23.4624                      |
| 2369                            | 19.8563                      |  | 2369                            | 23.6531                      |
| 2368                            | 20.0706                      |  | 2368                            | 24.2747                      |
| 2367                            | 19.7915                      |  | 2367                            | 23.8358                      |
| 2366                            | 20.1228                      |  | 2366                            | 23.918                       |
| 2365                            | 20.0702                      |  | 2365                            | 23.6427                      |
| 2364                            | 20.3577                      |  | 2364                            | 23.8159                      |
| 2363                            | 20.7976                      |  | 2363                            | 24.1554                      |
| 2362                            | 20.9194                      |  | 2362                            | 24.471                       |
| 2361                            | 21.5828                      |  | 2361                            | 24.957                       |

**FIG. 10**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2360                            | 21.2507                      |  | 2360                            | 24.4765                      |
| 2359                            | 21.3001                      |  | 2359                            | 24.6303                      |
| 2358                            | 21.4587                      |  | 2358                            | 24.5456                      |
| 2357                            | 21.279                       |  | 2357                            | 24.1122                      |
| 2356                            | 21.6741                      |  | 2356                            | 25.0556                      |
| 2355                            | 21.8272                      |  | 2355                            | 25.0168                      |
| 2354                            | 21.6811                      |  | 2354                            | 24.9495                      |
| 2353                            | 21.5385                      |  | 2353                            | 25.0189                      |
| 2352                            | 20.8254                      |  | 2352                            | 24.0242                      |
| 2351                            | 20.38                        |  | 2351                            | 23.5873                      |
| 2350                            | 20.3939                      |  | 2350                            | 23.8969                      |
| 2349                            | 20.2285                      |  | 2349                            | 23.1449                      |
| 2348                            | 20.5626                      |  | 2348                            | 23.3431                      |
| 2347                            | 20.525                       |  | 2347                            | 23.4015                      |
| 2346                            | 20.7342                      |  | 2346                            | 22.6203                      |
| 2345                            | 20.788                       |  | 2345                            | 23.513                       |
| 2344                            | 20.6299                      |  | 2344                            | 23.913                       |
| 2343                            | 20.6026                      |  | 2343                            | 23.7595                      |
| 2342                            | 19.9838                      |  | 2342                            | 24.2817                      |
| 2341                            | 19.9139                      |  | 2341                            | 23.8955                      |
| 2340                            | 19.7174                      |  | 2340                            | 23.1407                      |
| 2339                            | 19.6807                      |  | 2339                            | 23.0483                      |
| 2338                            | 19.9298                      |  | 2338                            | 23.0766                      |
| 2337                            | 20.2157                      |  | 2337                            | 23.3399                      |
| 2336                            | 20.7377                      |  | 2336                            | 23.5318                      |
| 2335                            | 20.9068                      |  | 2335                            | 23.6626                      |
| 2334                            | 21.0284                      |  | 2334                            | 23.2691                      |
| 2333                            | 21.4109                      |  | 2333                            | 23.5356                      |

**FIG. 11**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2332                            | 20.9074                      |  | 2332                            | 23.6446                      |
| 2331                            | 20.7828                      |  | 2331                            | 24.2648                      |
| 2330                            | 20.5085                      |  | 2330                            | 24.4612                      |
| 2329                            | 20.3125                      |  | 2329                            | 24.2236                      |
| 2328                            | 20.9489                      |  | 2328                            | 24.4012                      |
| 2327                            | 21.3958                      |  | 2327                            | 23.7635                      |
| 2326                            | 21.6204                      |  | 2326                            | 24.0707                      |
| 2325                            | 21.7234                      |  | 2325                            | 24.7447                      |
| 2324                            | 21.2935                      |  | 2324                            | 24.539                       |
| 2323                            | 20.7245                      |  | 2323                            | 24.8638                      |
| 2322                            | 20.7936                      |  | 2322                            | 24.6358                      |
| 2321                            | 20.7834                      |  | 2321                            | 23.5807                      |
| 2320                            | 20.2738                      |  | 2320                            | 23.2298                      |
| 2319                            | 20.3766                      |  | 2319                            | 22.8946                      |
| 2318                            | 20.6584                      |  | 2318                            | 23.2496                      |
| 2317                            | 20.4276                      |  | 2317                            | 23.151                       |
| 2316                            | 21.3083                      |  | 2316                            | 23.7172                      |
| 2315                            | 21.5201                      |  | 2315                            | 24.1345                      |
| 2314                            | 20.8412                      |  | 2314                            | 23.5321                      |
| 2313                            | 20.9711                      |  | 2313                            | 24.3244                      |
| 2312                            | 20.9053                      |  | 2312                            | 24.4165                      |
| 2311                            | 20.6776                      |  | 2311                            | 23.9165                      |
| 2310                            | 21.3309                      |  | 2310                            | 24.4806                      |
| 2309                            | 20.6673                      |  | 2309                            | 23.8407                      |
| 2308                            | 20.3517                      |  | 2308                            | 23.7826                      |
| 2307                            | 20.0835                      |  | 2307                            | 23.8282                      |
| 2306                            | 19.4491                      |  | 2306                            | 23.314                       |
| 2305                            | 19.4498                      |  | 2305                            | 23.4473                      |

## FIG. 12

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2304                            | 19.5903                      |  | 2304                            | 23.2497                      |
| 2303                            | 19.923                       |  | 2303                            | 23.5033                      |
| 2302                            | 19.7974                      |  | 2302                            | 23.4403                      |
| 2301                            | 20.7885                      |  | 2301                            | 24.1406                      |
| 2300                            | 20.8977                      |  | 2300                            | 24.3559                      |
| 2299                            | 20.8847                      |  | 2299                            | 24.2178                      |
| 2298                            | 21.3899                      |  | 2298                            | 24.6966                      |
| 2297                            | 20.532                       |  | 2297                            | 23.8195                      |
| 2296                            | 20.9205                      |  | 2296                            | 23.8428                      |
| 2295                            | 21.0043                      |  | 2295                            | 23.9705                      |
| 2294                            | 20.7663                      |  | 2294                            | 23.9715                      |
| 2293                            | 21.0782                      |  | 2293                            | 24.5141                      |
| 2292                            | 20.7582                      |  | 2292                            | 24.3739                      |
| 2291                            | 21.0841                      |  | 2291                            | 24.86                        |
| 2290                            | 21.1648                      |  | 2290                            | 25.1285                      |
| 2289                            | 21.0908                      |  | 2289                            | 24.9677                      |
| 2288                            | 20.8567                      |  | 2288                            | 24.9807                      |
| 2287                            | 20.4787                      |  | 2287                            | 24.5243                      |
| 2286                            | 20.3368                      |  | 2286                            | 23.8681                      |
| 2285                            | 20.3453                      |  | 2285                            | 23.6826                      |
| 2284                            | 20.6529                      |  | 2284                            | 24.1509                      |
| 2283                            | 20.2376                      |  | 2283                            | 23.9425                      |
| 2282                            | 20.6472                      |  | 2282                            | 24.3186                      |
| 2281                            | 20.7362                      |  | 2281                            | 24.6234                      |
| 2280                            | 20.3586                      |  | 2280                            | 24.1705                      |
| 2279                            | 20.9378                      |  | 2279                            | 24.5121                      |
| 2278                            | 20.7104                      |  | 2278                            | 24.5852                      |
| 2277                            | 20.4731                      |  | 2277                            | 24.3943                      |

## FIG. 13

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2276                            | 21.0378                      |  | 2276                            | 24.5359                      |
| 2275                            | 21.0506                      |  | 2275                            | 24.7063                      |
| 2274                            | 21.1796                      |  | 2274                            | 24.4749                      |
| 2273                            | 21.2443                      |  | 2273                            | 24.4558                      |
| 2272                            | 21.5269                      |  | 2272                            | 24.7852                      |
| 2271                            | 21.3231                      |  | 2271                            | 24.5263                      |
| 2270                            | 21.0024                      |  | 2270                            | 24.2692                      |
| 2269                            | 21.065                       |  | 2269                            | 24.2144                      |
| 2268                            | 20.619                       |  | 2268                            | 23.7959                      |
| 2267                            | 20.9962                      |  | 2267                            | 23.8979                      |
| 2266                            | 20.9343                      |  | 2266                            | 24.1589                      |
| 2265                            | 21.0734                      |  | 2265                            | 24.2938                      |
| 2264                            | 21.0484                      |  | 2264                            | 24.5203                      |
| 2263                            | 21.1419                      |  | 2263                            | 24.3866                      |
| 2262                            | 21.4877                      |  | 2262                            | 24.3079                      |
| 2261                            | 21.27                        |  | 2261                            | 24.0722                      |
| 2260                            | 21.2349                      |  | 2260                            | 24.3002                      |
| 2259                            | 20.7669                      |  | 2259                            | 24.428                       |
| 2258                            | 20.8053                      |  | 2258                            | 24.7736                      |
| 2257                            | 21.0872                      |  | 2257                            | 24.9529                      |
| 2256                            | 21.2075                      |  | 2256                            | 24.6165                      |
| 2255                            | 21.3271                      |  | 2255                            | 24.544                       |
| 2254                            | 21.274                       |  | 2254                            | 24.3092                      |
| 2253                            | 20.938                       |  | 2253                            | 24.1621                      |
| 2252                            | 20.5832                      |  | 2252                            | 24.1008                      |
| 2251                            | 20.6211                      |  | 2251                            | 24.3633                      |
| 2250                            | 20.2975                      |  | 2250                            | 24.1308                      |
| 2249                            | 20.5318                      |  | 2249                            | 24.477                       |

**FIG. 14**

| Tape in black                   |                              | Tape in white                   |                              |
|---------------------------------|------------------------------|---------------------------------|------------------------------|
| Wavelength<br>( $\mu\text{m}$ ) | Light transmittance<br>T (%) | Wavelength<br>( $\mu\text{m}$ ) | Light transmittance T<br>(%) |
| 2248                            | 21.0266                      | 2248                            | 24.6103                      |
| 2247                            | 20.966                       | 2247                            | 24.3094                      |
| 2246                            | 21.2804                      | 2246                            | 24.8749                      |
| 2245                            | 21.0883                      | 2245                            | 24.3059                      |
| 2244                            | 20.6847                      | 2244                            | 24.3209                      |
| 2243                            | 20.578                       | 2243                            | 24.2085                      |
| 2242                            | 20.2154                      | 2242                            | 23.9079                      |
| 2241                            | 20.28                        | 2241                            | 24.1615                      |
| 2240                            | 20.1226                      | 2240                            | 23.9188                      |
| 2239                            | 20.0905                      | 2239                            | 24.2986                      |
| 2238                            | 20.6671                      | 2238                            | 24.1682                      |
| 2237                            | 20.5352                      | 2237                            | 24.034                       |
| 2236                            | 20.9557                      | 2236                            | 24.2114                      |
| 2235                            | 21.1962                      | 2235                            | 24.324                       |
| 2234                            | 21.1383                      | 2234                            | 24.461                       |
| 2233                            | 21.5334                      | 2233                            | 24.9732                      |
| 2232                            | 21.3113                      | 2232                            | 24.7124                      |
| 2231                            | 21.0479                      | 2231                            | 24.1391                      |
| 2230                            | 20.7994                      | 2230                            | 24.1372                      |
| 2229                            | 21.027                       | 2229                            | 24.2002                      |
| 2228                            | 20.8491                      | 2228                            | 24.1876                      |
| 2227                            | 20.9924                      | 2227                            | 24.4604                      |
| 2226                            | 20.98                        | 2226                            | 24.347                       |
| 2225                            | 20.6796                      | 2225                            | 24.2126                      |
| 2224                            | 21.0663                      | 2224                            | 24.3084                      |
| 2223                            | 21.2915                      | 2223                            | 24.6032                      |
| 2222                            | 21.6494                      | 2222                            | 24.9106                      |

## FIG. 15

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2221                            | 21.739                       |  | 2221                            | 24.59                        |
| 2220                            | 21.7319                      |  | 2220                            | 24.6605                      |
| 2219                            | 21.9349                      |  | 2219                            | 24.365                       |
| 2218                            | 21.4854                      |  | 2218                            | 24.1716                      |
| 2217                            | 21.401                       |  | 2217                            | 24.3209                      |
| 2216                            | 21.3938                      |  | 2216                            | 24.4352                      |
| 2215                            | 20.9786                      |  | 2215                            | 24.4223                      |
| 2214                            | 21.0878                      |  | 2214                            | 24.3851                      |
| 2213                            | 21.2351                      |  | 2213                            | 24.4697                      |
| 2212                            | 21.0495                      |  | 2212                            | 24.2946                      |
| 2211                            | 21.2019                      |  | 2211                            | 24.5232                      |
| 2210                            | 21.1621                      |  | 2210                            | 24.5405                      |
| 2209                            | 20.8989                      |  | 2209                            | 24.1911                      |
| 2208                            | 21.0841                      |  | 2208                            | 24.2035                      |
| 2207                            | 21.1156                      |  | 2207                            | 24.0076                      |
| 2206                            | 21.2798                      |  | 2206                            | 24.2996                      |
| 2205                            | 21.2973                      |  | 2205                            | 24.7133                      |
| 2204                            | 21.134                       |  | 2204                            | 24.8501                      |
| 2203                            | 21.0783                      |  | 2203                            | 25.0088                      |
| 2202                            | 21.0813                      |  | 2202                            | 24.8168                      |
| 2201                            | 21.3669                      |  | 2201                            | 24.8349                      |
| 2200                            | 21.3683                      |  | 2200                            | 24.7434                      |
| 2199                            | 21.1331                      |  | 2199                            | 24.6222                      |
| 2198                            | 21.194                       |  | 2198                            | 25.035                       |
| 2197                            | 20.6622                      |  | 2197                            | 24.7686                      |
| 2196                            | 20.822                       |  | 2196                            | 24.7402                      |
| 2195                            | 21.2599                      |  | 2195                            | 24.8583                      |
| 2194                            | 20.9169                      |  | 2194                            | 24.3991                      |

## FIG. 16

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2193                            | 21.1561                      |  | 2193                            | 24.6642                      |
| 2192                            | 21.1678                      |  | 2192                            | 24.852                       |
| 2191                            | 20.8938                      |  | 2191                            | 24.5874                      |
| 2190                            | 20.9954                      |  | 2190                            | 24.4113                      |
| 2189                            | 20.9154                      |  | 2189                            | 24.2536                      |
| 2188                            | 21.0807                      |  | 2188                            | 24.1037                      |
| 2187                            | 21.4344                      |  | 2187                            | 24.5073                      |
| 2186                            | 21.4304                      |  | 2186                            | 24.519                       |
| 2185                            | 21.3336                      |  | 2185                            | 24.6033                      |
| 2184                            | 20.9671                      |  | 2184                            | 24.6343                      |
| 2183                            | 20.7242                      |  | 2183                            | 24.4656                      |
| 2182                            | 20.9186                      |  | 2182                            | 24.752                       |
| 2181                            | 21.0932                      |  | 2181                            | 24.61                        |
| 2180                            | 21.1881                      |  | 2180                            | 24.528                       |
| 2179                            | 21.3579                      |  | 2179                            | 24.689                       |
| 2178                            | 21.4244                      |  | 2178                            | 24.5917                      |
| 2177                            | 21.6347                      |  | 2177                            | 24.9473                      |
| 2176                            | 21.7124                      |  | 2176                            | 25.0891                      |
| 2175                            | 21.3713                      |  | 2175                            | 24.7088                      |
| 2174                            | 21.1551                      |  | 2174                            | 24.7659                      |
| 2173                            | 20.9774                      |  | 2173                            | 24.6676                      |
| 2172                            | 20.7269                      |  | 2172                            | 24.4345                      |
| 2171                            | 21.1614                      |  | 2171                            | 24.8455                      |
| 2170                            | 21.1854                      |  | 2170                            | 24.7629                      |
| 2169                            | 21.443                       |  | 2169                            | 24.8017                      |
| 2168                            | 21.4863                      |  | 2168                            | 24.943                       |
| 2167                            | 21.3961                      |  | 2167                            | 24.8015                      |
| 2166                            | 21.5504                      |  | 2166                            | 25.1282                      |

## FIG. 17

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2165                            | 21.2845                      |  | 2165                            | 24.7927                      |
| 2164                            | 21.322                       |  | 2164                            | 24.7083                      |
| 2163                            | 21.0036                      |  | 2163                            | 24.7362                      |
| 2162                            | 21.0132                      |  | 2162                            | 24.2949                      |
| 2161                            | 20.9858                      |  | 2161                            | 24.4622                      |
| 2160                            | 20.8878                      |  | 2160                            | 24.4591                      |
| 2159                            | 21.0863                      |  | 2159                            | 24.3782                      |
| 2158                            | 20.718                       |  | 2158                            | 24.3008                      |
| 2157                            | 20.667                       |  | 2157                            | 24.468                       |
| 2156                            | 21.0471                      |  | 2156                            | 24.6297                      |
| 2155                            | 20.847                       |  | 2155                            | 24.3951                      |
| 2154                            | 21.212                       |  | 2154                            | 24.5981                      |
| 2153                            | 21.1375                      |  | 2153                            | 24.444                       |
| 2152                            | 20.8854                      |  | 2152                            | 24.4261                      |
| 2151                            | 20.9512                      |  | 2151                            | 24.576                       |
| 2150                            | 20.5029                      |  | 2150                            | 24.4445                      |
| 2149                            | 20.5556                      |  | 2149                            | 24.3567                      |
| 2148                            | 20.7318                      |  | 2148                            | 24.7211                      |
| 2147                            | 20.917                       |  | 2147                            | 24.6226                      |
| 2146                            | 21.4453                      |  | 2146                            | 25.1753                      |
| 2145                            | 21.5451                      |  | 2145                            | 25.2516                      |
| 2144                            | 21.2841                      |  | 2144                            | 24.8536                      |
| 2143                            | 21.165                       |  | 2143                            | 24.8932                      |
| 2142                            | 20.9042                      |  | 2142                            | 24.4635                      |
| 2141                            | 20.9827                      |  | 2141                            | 24.39                        |
| 2140                            | 20.9551                      |  | 2140                            | 24.304                       |
| 2139                            | 21.1972                      |  | 2139                            | 24.4808                      |
| 2138                            | 21.2293                      |  | 2138                            | 24.3779                      |

**FIG. 18**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2137                            | 21.1843                      |  | 2137                            | 24.5521                      |
| 2136                            | 21.3941                      |  | 2136                            | 24.6033                      |
| 2135                            | 21.1678                      |  | 2135                            | 24.7492                      |
| 2134                            | 21.1175                      |  | 2134                            | 24.7473                      |
| 2133                            | 21.1165                      |  | 2133                            | 24.6172                      |
| 2132                            | 21.077                       |  | 2132                            | 24.7495                      |
| 2131                            | 20.724                       |  | 2131                            | 24.3356                      |
| 2130                            | 20.9017                      |  | 2130                            | 24.4468                      |
| 2129                            | 20.7677                      |  | 2129                            | 24.4312                      |
| 2128                            | 20.7191                      |  | 2128                            | 24.5115                      |
| 2127                            | 20.7815                      |  | 2127                            | 24.4472                      |
| 2126                            | 20.7893                      |  | 2126                            | 24.5267                      |
| 2125                            | 20.7844                      |  | 2125                            | 24.4792                      |
| 2124                            | 20.9753                      |  | 2124                            | 24.4889                      |
| 2123                            | 21.1438                      |  | 2123                            | 24.6159                      |
| 2122                            | 20.9852                      |  | 2122                            | 24.5771                      |
| 2121                            | 21.1169                      |  | 2121                            | 24.7                         |
| 2120                            | 20.9305                      |  | 2120                            | 24.4388                      |
| 2119                            | 20.9478                      |  | 2119                            | 24.5155                      |
| 2118                            | 21.0354                      |  | 2118                            | 24.5821                      |
| 2117                            | 21.1345                      |  | 2117                            | 24.8046                      |
| 2116                            | 21.2793                      |  | 2116                            | 24.8856                      |
| 2115                            | 21.3739                      |  | 2115                            | 24.8859                      |
| 2114                            | 21.4149                      |  | 2114                            | 24.8068                      |
| 2113                            | 21.1322                      |  | 2113                            | 24.4064                      |
| 2112                            | 20.9921                      |  | 2112                            | 24.3037                      |
| 2111                            | 20.7892                      |  | 2111                            | 24.3688                      |
| 2110                            | 20.7121                      |  | 2110                            | 24.349                       |

## FIG. 19

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2109                            | 20.5771                      |  | 2109                            | 24.3032                      |
| 2108                            | 20.502                       |  | 2108                            | 24.4479                      |
| 2107                            | 20.7473                      |  | 2107                            | 24.5782                      |
| 2106                            | 20.4867                      |  | 2106                            | 24.1888                      |
| 2105                            | 20.7703                      |  | 2105                            | 24.3183                      |
| 2104                            | 20.9829                      |  | 2104                            | 24.2998                      |
| 2103                            | 21.0966                      |  | 2103                            | 24.3098                      |
| 2102                            | 21.4666                      |  | 2102                            | 24.5597                      |
| 2101                            | 21.6078                      |  | 2101                            | 24.7905                      |
| 2100                            | 21.4975                      |  | 2100                            | 24.9012                      |
| 2099                            | 21.4346                      |  | 2099                            | 24.9261                      |
| 2098                            | 21.5033                      |  | 2098                            | 25.0906                      |
| 2097                            | 21.4117                      |  | 2097                            | 24.9968                      |
| 2096                            | 21.3047                      |  | 2096                            | 24.7065                      |
| 2095                            | 20.9488                      |  | 2095                            | 24.6249                      |
| 2094                            | 21.0654                      |  | 2094                            | 24.6595                      |
| 2093                            | 21.1371                      |  | 2093                            | 24.5306                      |
| 2092                            | 21.4131                      |  | 2092                            | 24.9098                      |
| 2091                            | 21.7275                      |  | 2091                            | 24.8311                      |
| 2090                            | 21.4534                      |  | 2090                            | 24.7392                      |
| 2089                            | 21.4208                      |  | 2089                            | 24.6816                      |
| 2088                            | 21.2651                      |  | 2088                            | 24.4945                      |
| 2087                            | 21.4546                      |  | 2087                            | 24.6233                      |
| 2086                            | 21.6158                      |  | 2086                            | 24.8277                      |
| 2085                            | 21.5569                      |  | 2085                            | 24.9769                      |
| 2084                            | 21.4215                      |  | 2084                            | 24.7776                      |
| 2083                            | 21.2015                      |  | 2083                            | 24.6209                      |
| 2082                            | 21.0095                      |  | 2082                            | 24.3854                      |

**FIG. 20**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2081                            | 21.1537                      |  | 2081                            | 24.5276                      |
| 2080                            | 20.9984                      |  | 2080                            | 24.6163                      |
| 2079                            | 21.0256                      |  | 2079                            | 24.6774                      |
| 2078                            | 21.2263                      |  | 2078                            | 25.0046                      |
| 2077                            | 21.041                       |  | 2077                            | 24.8714                      |
| 2076                            | 21.0851                      |  | 2076                            | 24.9393                      |
| 2075                            | 20.8657                      |  | 2075                            | 24.8529                      |
| 2074                            | 20.7712                      |  | 2074                            | 24.6606                      |
| 2073                            | 20.9159                      |  | 2073                            | 24.7585                      |
| 2072                            | 21.1648                      |  | 2072                            | 24.6411                      |
| 2071                            | 21.4115                      |  | 2071                            | 24.7535                      |
| 2070                            | 21.5081                      |  | 2070                            | 24.9278                      |
| 2069                            | 21.4864                      |  | 2069                            | 24.8313                      |
| 2068                            | 21.5564                      |  | 2068                            | 25.0473                      |
| 2067                            | 21.5029                      |  | 2067                            | 25.1645                      |
| 2066                            | 21.3761                      |  | 2066                            | 24.9916                      |
| 2065                            | 21.3489                      |  | 2065                            | 24.8773                      |
| 2064                            | 21.3133                      |  | 2064                            | 24.7313                      |
| 2063                            | 21.2913                      |  | 2063                            | 24.6309                      |
| 2062                            | 21.2603                      |  | 2062                            | 24.4927                      |
| 2061                            | 21.3211                      |  | 2061                            | 24.5134                      |
| 2060                            | 21.3001                      |  | 2060                            | 24.5281                      |
| 2059                            | 21.5281                      |  | 2059                            | 24.59                        |
| 2058                            | 21.483                       |  | 2058                            | 24.8127                      |
| 2057                            | 21.1269                      |  | 2057                            | 24.7532                      |
| 2056                            | 21.034                       |  | 2056                            | 24.7682                      |
| 2055                            | 20.9212                      |  | 2055                            | 24.8206                      |
| 2054                            | 20.9298                      |  | 2054                            | 24.6181                      |

## FIG. 21

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2053                            | 21.1377                      |  | 2053                            | 24.7847                      |
| 2052                            | 21.1069                      |  | 2052                            | 24.6699                      |
| 2051                            | 21.0036                      |  | 2051                            | 24.4762                      |
| 2050                            | 20.8672                      |  | 2050                            | 24.6254                      |
| 2049                            | 20.8459                      |  | 2049                            | 24.5248                      |
| 2048                            | 20.9273                      |  | 2048                            | 24.7721                      |
| 2047                            | 21.087                       |  | 2047                            | 24.8386                      |
| 2046                            | 21.221                       |  | 2046                            | 24.9289                      |
| 2045                            | 21.305                       |  | 2045                            | 25.0052                      |
| 2044                            | 21.0497                      |  | 2044                            | 24.7347                      |
| 2043                            | 20.9455                      |  | 2043                            | 24.8092                      |
| 2042                            | 20.9666                      |  | 2042                            | 24.5881                      |
| 2041                            | 20.8722                      |  | 2041                            | 24.5402                      |
| 2040                            | 21.157                       |  | 2040                            | 24.7489                      |
| 2039                            | 20.982                       |  | 2039                            | 24.6468                      |
| 2038                            | 20.9815                      |  | 2038                            | 24.5375                      |
| 2037                            | 21.0093                      |  | 2037                            | 24.545                       |
| 2036                            | 20.9845                      |  | 2036                            | 24.507                       |
| 2035                            | 21.1242                      |  | 2035                            | 24.4848                      |
| 2034                            | 21.1936                      |  | 2034                            | 24.5219                      |
| 2033                            | 21.2468                      |  | 2033                            | 24.6159                      |
| 2032                            | 21.3202                      |  | 2032                            | 24.8488                      |
| 2031                            | 21.3119                      |  | 2031                            | 25.0328                      |
| 2030                            | 21.3788                      |  | 2030                            | 25.2742                      |
| 2029                            | 21.3492                      |  | 2029                            | 25.0584                      |
| 2028                            | 21.1692                      |  | 2028                            | 24.7934                      |
| 2027                            | 21.019                       |  | 2027                            | 24.6261                      |
| 2026                            | 20.655                       |  | 2026                            | 24.4226                      |

## FIG. 22

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 2025                            | 20.6259                      |  | 2025                            | 24.6568                      |
| 2024                            | 20.7063                      |  | 2024                            | 24.7931                      |
| 2023                            | 20.7067                      |  | 2023                            | 24.6528                      |
| 2022                            | 21.0512                      |  | 2022                            | 24.7997                      |
| 2021                            | 20.9372                      |  | 2021                            | 24.6129                      |
| 2020                            | 21.0328                      |  | 2020                            | 24.3265                      |
| 2019                            | 21.069                       |  | 2019                            | 24.3857                      |
| 2018                            | 21.0402                      |  | 2018                            | 24.5133                      |
| 2017                            | 21.1792                      |  | 2017                            | 24.761                       |
| 2016                            | 21.0113                      |  | 2016                            | 24.9049                      |
| 2015                            | 21.2701                      |  | 2015                            | 25.0833                      |
| 2014                            | 21.2432                      |  | 2014                            | 24.907                       |
| 2013                            | 21.3702                      |  | 2013                            | 24.8395                      |
| 2012                            | 21.6018                      |  | 2012                            | 25.0435                      |
| 2011                            | 21.5318                      |  | 2011                            | 24.8566                      |
| 2010                            | 21.3891                      |  | 2010                            | 24.7506                      |
| 2009                            | 21.3088                      |  | 2009                            | 24.7016                      |
| 2008                            | 21.2215                      |  | 2008                            | 24.7223                      |
| 2007                            | 21.3684                      |  | 2007                            | 24.8457                      |
| 2006                            | 21.6003                      |  | 2006                            | 25.1532                      |
| 2005                            | 21.5502                      |  | 2005                            | 25.1535                      |
| 2004                            | 21.7191                      |  | 2004                            | 25.26                        |
| 2003                            | 21.6505                      |  | 2003                            | 25.0906                      |
| 2002                            | 21.6741                      |  | 2002                            | 25.0041                      |
| 2001                            | 21.5463                      |  | 2001                            | 24.8988                      |
| 2000                            | 21.2829                      |  | 2000                            | 24.716                       |
| 1999                            | 21.0841                      |  | 1999                            | 24.774                       |
| 1998                            | 20.8336                      |  | 1998                            | 24.6161                      |

## FIG. 23

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1997                            | 20.9435                      |  | 1997                            | 24.525                       |
| 1996                            | 20.8853                      |  | 1996                            | 24.467                       |
| 1995                            | 20.829                       |  | 1995                            | 24.5197                      |
| 1994                            | 21.0328                      |  | 1994                            | 24.5684                      |
| 1993                            | 20.9742                      |  | 1993                            | 24.7013                      |
| 1992                            | 21.173                       |  | 1992                            | 24.8217                      |
| 1991                            | 21.1715                      |  | 1991                            | 24.817                       |
| 1990                            | 20.8458                      |  | 1990                            | 24.6569                      |
| 1989                            | 20.924                       |  | 1989                            | 24.8348                      |
| 1988                            | 21.0217                      |  | 1988                            | 24.7504                      |
| 1987                            | 21.1075                      |  | 1987                            | 24.8016                      |
| 1986                            | 21.4558                      |  | 1986                            | 24.9988                      |
| 1985                            | 21.4501                      |  | 1985                            | 24.8311                      |
| 1984                            | 21.2761                      |  | 1984                            | 24.7278                      |
| 1983                            | 21.1289                      |  | 1983                            | 24.7184                      |
| 1982                            | 21.0876                      |  | 1982                            | 24.7098                      |
| 1981                            | 21.0266                      |  | 1981                            | 24.7005                      |
| 1980                            | 20.9575                      |  | 1980                            | 24.8245                      |
| 1979                            | 21.0181                      |  | 1979                            | 24.7916                      |
| 1978                            | 20.7554                      |  | 1978                            | 24.6445                      |
| 1977                            | 20.7771                      |  | 1977                            | 24.6534                      |
| 1976                            | 20.6121                      |  | 1976                            | 24.3281                      |
| 1975                            | 20.7154                      |  | 1975                            | 24.3953                      |
| 1974                            | 20.8741                      |  | 1974                            | 24.4011                      |
| 1973                            | 20.9722                      |  | 1973                            | 24.8146                      |
| 1972                            | 21.1165                      |  | 1972                            | 24.6819                      |
| 1971                            | 21.104                       |  | 1971                            | 24.5342                      |
| 1970                            | 21.1632                      |  | 1970                            | 24.6656                      |

**FIG. 24**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1969                            | 21.0993                      |  | 1969                            | 24.8437                      |
| 1968                            | 21.0262                      |  | 1968                            | 24.7747                      |
| 1967                            | 21.0831                      |  | 1967                            | 24.7926                      |
| 1966                            | 20.9673                      |  | 1966                            | 24.8541                      |
| 1965                            | 21.0636                      |  | 1965                            | 24.8451                      |
| 1964                            | 21.0566                      |  | 1964                            | 24.7635                      |
| 1963                            | 20.8102                      |  | 1963                            | 24.7573                      |
| 1962                            | 20.9966                      |  | 1962                            | 24.7321                      |
| 1961                            | 20.6477                      |  | 1961                            | 24.3573                      |
| 1960                            | 20.9791                      |  | 1960                            | 24.6421                      |
| 1959                            | 21.1892                      |  | 1959                            | 24.7354                      |
| 1958                            | 21.208                       |  | 1958                            | 24.7463                      |
| 1957                            | 21.5266                      |  | 1957                            | 25.027                       |
| 1956                            | 21.5258                      |  | 1956                            | 24.773                       |
| 1955                            | 21.5415                      |  | 1955                            | 24.7675                      |
| 1954                            | 21.3398                      |  | 1954                            | 24.653                       |
| 1953                            | 21.217                       |  | 1953                            | 24.633                       |
| 1952                            | 21.2972                      |  | 1952                            | 24.7737                      |
| 1951                            | 21.2375                      |  | 1951                            | 24.703                       |
| 1950                            | 21.2332                      |  | 1950                            | 24.6199                      |
| 1949                            | 21.3206                      |  | 1949                            | 24.7608                      |
| 1948                            | 21.0799                      |  | 1948                            | 24.6995                      |
| 1947                            | 21.2923                      |  | 1947                            | 24.8988                      |
| 1946                            | 21.4834                      |  | 1946                            | 25.022                       |
| 1945                            | 21.4328                      |  | 1945                            | 24.9274                      |
| 1944                            | 21.5766                      |  | 1944                            | 24.9309                      |
| 1943                            | 21.4537                      |  | 1943                            | 24.5683                      |
| 1942                            | 21.3339                      |  | 1942                            | 24.6215                      |

## FIG. 25

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1941                            | 21.4006                      |  | 1941                            | 24.7051                      |
| 1940                            | 21.0915                      |  | 1940                            | 24.6533                      |
| 1939                            | 20.8588                      |  | 1939                            | 24.759                       |
| 1938                            | 20.9445                      |  | 1938                            | 24.799                       |
| 1937                            | 21.1827                      |  | 1937                            | 24.838                       |
| 1936                            | 21.4243                      |  | 1936                            | 24.6959                      |
| 1935                            | 21.6742                      |  | 1935                            | 24.8704                      |
| 1934                            | 21.6741                      |  | 1934                            | 24.779                       |
| 1933                            | 21.5097                      |  | 1933                            | 24.7467                      |
| 1932                            | 21.3606                      |  | 1932                            | 24.6701                      |
| 1931                            | 21.2925                      |  | 1931                            | 24.5067                      |
| 1930                            | 21.024                       |  | 1930                            | 24.3102                      |
| 1929                            | 21.0434                      |  | 1929                            | 24.4785                      |
| 1928                            | 21.1717                      |  | 1928                            | 24.7671                      |
| 1927                            | 21.2591                      |  | 1927                            | 24.9314                      |
| 1926                            | 21.7043                      |  | 1926                            | 25.4041                      |
| 1925                            | 21.6021                      |  | 1925                            | 25.1286                      |
| 1924                            | 21.5362                      |  | 1924                            | 25.0402                      |
| 1923                            | 21.4829                      |  | 1923                            | 24.9174                      |
| 1922                            | 21.2538                      |  | 1922                            | 24.701                       |
| 1921                            | 21.3979                      |  | 1921                            | 24.7563                      |
| 1920                            | 21.2423                      |  | 1920                            | 24.5728                      |
| 1919                            | 21.1616                      |  | 1919                            | 24.7628                      |
| 1918                            | 21.2155                      |  | 1918                            | 24.7965                      |
| 1917                            | 20.9734                      |  | 1917                            | 24.6356                      |
| 1916                            | 21.1923                      |  | 1916                            | 24.8685                      |
| 1915                            | 21.1104                      |  | 1915                            | 24.6923                      |
| 1914                            | 21.0669                      |  | 1914                            | 24.809                       |

## FIG. 26

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1913                            | 21.1681                      |  | 1913                            | 24.97                        |
| 1912                            | 21.1772                      |  | 1912                            | 24.9326                      |
| 1911                            | 21.1837                      |  | 1911                            | 24.8689                      |
| 1910                            | 21.1592                      |  | 1910                            | 24.7287                      |
| 1909                            | 21.1089                      |  | 1909                            | 24.7336                      |
| 1908                            | 21.0951                      |  | 1908                            | 24.8697                      |
| 1907                            | 21.3047                      |  | 1907                            | 25.0031                      |
| 1906                            | 21.2821                      |  | 1906                            | 25.1329                      |
| 1905                            | 21.3778                      |  | 1905                            | 25.2247                      |
| 1904                            | 21.5506                      |  | 1904                            | 25.1587                      |
| 1903                            | 21.4111                      |  | 1903                            | 25.1876                      |
| 1902                            | 21.1554                      |  | 1902                            | 25.0332                      |
| 1901                            | 21.2555                      |  | 1901                            | 25.0907                      |
| 1900                            | 21.4408                      |  | 1900                            | 25.1434                      |
| 1899                            | 21.4826                      |  | 1899                            | 25.2486                      |
| 1898                            | 21.6029                      |  | 1898                            | 25.3284                      |
| 1897                            | 21.7249                      |  | 1897                            | 25.4373                      |
| 1896                            | 21.5431                      |  | 1896                            | 25.2631                      |
| 1895                            | 21.6422                      |  | 1895                            | 25.3051                      |
| 1894                            | 21.4903                      |  | 1894                            | 25.1655                      |
| 1893                            | 21.3753                      |  | 1893                            | 24.9502                      |
| 1892                            | 21.6422                      |  | 1892                            | 25.0706                      |
| 1891                            | 21.6542                      |  | 1891                            | 24.9753                      |
| 1890                            | 21.8053                      |  | 1890                            | 25.0701                      |
| 1889                            | 21.8711                      |  | 1889                            | 25.0434                      |
| 1888                            | 21.6653                      |  | 1888                            | 25.0441                      |
| 1887                            | 21.6383                      |  | 1887                            | 25.0535                      |
| 1886                            | 21.4899                      |  | 1886                            | 25.0099                      |

## FIG. 27

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1885                            | 21.4702                      |  | 1885                            | 25.0359                      |
| 1884                            | 21.5366                      |  | 1884                            | 25.0733                      |
| 1883                            | 21.4699                      |  | 1883                            | 25.0886                      |
| 1882                            | 21.5176                      |  | 1882                            | 25.089                       |
| 1881                            | 21.5031                      |  | 1881                            | 25.0273                      |
| 1880                            | 21.456                       |  | 1880                            | 25.0697                      |
| 1879                            | 21.4424                      |  | 1879                            | 25.0308                      |
| 1878                            | 21.3433                      |  | 1878                            | 24.9266                      |
| 1877                            | 21.3959                      |  | 1877                            | 25.0396                      |
| 1876                            | 21.4535                      |  | 1876                            | 24.8529                      |
| 1875                            | 21.485                       |  | 1875                            | 24.8787                      |
| 1874                            | 21.6129                      |  | 1874                            | 24.9298                      |
| 1873                            | 21.5378                      |  | 1873                            | 24.9067                      |
| 1872                            | 21.5788                      |  | 1872                            | 25.0131                      |
| 1871                            | 21.5897                      |  | 1871                            | 24.8682                      |
| 1870                            | 21.5482                      |  | 1870                            | 24.9319                      |
| 1869                            | 21.3987                      |  | 1869                            | 24.7877                      |
| 1868                            | 21.2545                      |  | 1868                            | 24.7042                      |
| 1867                            | 21.1184                      |  | 1867                            | 24.9215                      |
| 1866                            | 21.1051                      |  | 1866                            | 24.8658                      |
| 1865                            | 21.2395                      |  | 1865                            | 25.0456                      |
| 1864                            | 21.288                       |  | 1864                            | 25.0659                      |
| 1863                            | 21.3768                      |  | 1863                            | 24.9638                      |
| 1862                            | 21.3051                      |  | 1862                            | 24.9847                      |
| 1861                            | 21.2309                      |  | 1861                            | 24.9013                      |
| 1860                            | 21.2488                      |  | 1860                            | 24.9878                      |
| 1859                            | 21.2235                      |  | 1859                            | 24.9658                      |
| 1858                            | 21.2741                      |  | 1858                            | 24.955                       |

## FIG. 28

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1857                            | 21.4194                      |  | 1857                            | 24.9248                      |
| 1856                            | 21.4783                      |  | 1856                            | 24.8845                      |
| 1855                            | 21.4882                      |  | 1855                            | 24.9545                      |
| 1854                            | 21.557                       |  | 1854                            | 25.0132                      |
| 1853                            | 21.4707                      |  | 1853                            | 24.9974                      |
| 1852                            | 21.4236                      |  | 1852                            | 24.9654                      |
| 1851                            | 21.4167                      |  | 1851                            | 24.8799                      |
| 1850                            | 21.1914                      |  | 1850                            | 24.8133                      |
| 1849                            | 21.336                       |  | 1849                            | 24.9458                      |
| 1848                            | 21.2787                      |  | 1848                            | 24.9886                      |
| 1847                            | 21.3297                      |  | 1847                            | 25.1078                      |
| 1846                            | 21.4755                      |  | 1846                            | 25.134                       |
| 1845                            | 21.3613                      |  | 1845                            | 25.1093                      |
| 1844                            | 21.4046                      |  | 1844                            | 25.0256                      |
| 1843                            | 21.3526                      |  | 1843                            | 24.9892                      |
| 1842                            | 21.3622                      |  | 1842                            | 24.9816                      |
| 1841                            | 21.3688                      |  | 1841                            | 24.8762                      |
| 1840                            | 21.3733                      |  | 1840                            | 24.9093                      |
| 1839                            | 21.3745                      |  | 1839                            | 24.8216                      |
| 1838                            | 21.372                       |  | 1838                            | 24.7867                      |
| 1837                            | 21.3399                      |  | 1837                            | 24.793                       |
| 1836                            | 21.3009                      |  | 1836                            | 24.8382                      |
| 1835                            | 21.3148                      |  | 1835                            | 24.8431                      |
| 1834                            | 21.4117                      |  | 1834                            | 24.9222                      |
| 1833                            | 21.4174                      |  | 1833                            | 24.9568                      |
| 1832                            | 21.5124                      |  | 1832                            | 24.9545                      |
| 1831                            | 21.512                       |  | 1831                            | 24.9602                      |
| 1830                            | 21.3904                      |  | 1830                            | 24.8363                      |

## FIG. 29

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1829                            | 21.4519                      |  | 1829                            | 24.8368                      |
| 1828                            | 21.4509                      |  | 1828                            | 24.9001                      |
| 1827                            | 21.4569                      |  | 1827                            | 24.9266                      |
| 1826                            | 21.5329                      |  | 1826                            | 24.9766                      |
| 1825                            | 21.4814                      |  | 1825                            | 24.97                        |
| 1824                            | 21.3931                      |  | 1824                            | 24.9179                      |
| 1823                            | 21.4217                      |  | 1823                            | 24.9714                      |
| 1822                            | 21.3642                      |  | 1822                            | 25.01                        |
| 1821                            | 21.3855                      |  | 1821                            | 25.0839                      |
| 1820                            | 21.3673                      |  | 1820                            | 25.0277                      |
| 1819                            | 21.3519                      |  | 1819                            | 25.028                       |
| 1818                            | 21.3739                      |  | 1818                            | 24.989                       |
| 1817                            | 21.4063                      |  | 1817                            | 24.9106                      |
| 1816                            | 21.408                       |  | 1816                            | 24.9117                      |
| 1815                            | 21.4511                      |  | 1815                            | 24.8954                      |
| 1814                            | 21.4247                      |  | 1814                            | 24.9279                      |
| 1813                            | 21.4212                      |  | 1813                            | 24.9577                      |
| 1812                            | 21.5235                      |  | 1812                            | 24.9922                      |
| 1811                            | 21.4695                      |  | 1811                            | 24.9536                      |
| 1810                            | 21.5783                      |  | 1810                            | 24.961                       |
| 1809                            | 21.6174                      |  | 1809                            | 24.9625                      |
| 1808                            | 21.5926                      |  | 1808                            | 25.001                       |
| 1807                            | 21.6359                      |  | 1807                            | 25.003                       |
| 1806                            | 21.5098                      |  | 1806                            | 24.9134                      |
| 1805                            | 21.4947                      |  | 1805                            | 24.9349                      |
| 1804                            | 21.5428                      |  | 1804                            | 24.9886                      |
| 1803                            | 21.4879                      |  | 1803                            | 25.0366                      |
| 1802                            | 21.5612                      |  | 1802                            | 25.1413                      |

## FIG. 30

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1801                            | 21.515                       |  | 1801                            | 25.1636                      |
| 1800                            | 21.5305                      |  | 1800                            | 25.1118                      |
| 1799                            | 21.648                       |  | 1799                            | 25.1387                      |
| 1798                            | 21.6547                      |  | 1798                            | 25.1578                      |
| 1797                            | 21.6736                      |  | 1797                            | 25.1266                      |
| 1796                            | 21.6123                      |  | 1796                            | 25.0772                      |
| 1795                            | 21.5264                      |  | 1795                            | 25.059                       |
| 1794                            | 21.4879                      |  | 1794                            | 25.0096                      |
| 1793                            | 21.5071                      |  | 1793                            | 24.991                       |
| 1792                            | 21.5058                      |  | 1792                            | 25.0102                      |
| 1791                            | 21.5538                      |  | 1791                            | 24.9934                      |
| 1790                            | 21.5752                      |  | 1790                            | 25.0742                      |
| 1789                            | 21.5731                      |  | 1789                            | 25.1193                      |
| 1788                            | 21.6523                      |  | 1788                            | 25.1171                      |
| 1787                            | 21.6297                      |  | 1787                            | 25.1165                      |
| 1786                            | 21.647                       |  | 1786                            | 25.0664                      |
| 1785                            | 21.6494                      |  | 1785                            | 25.0668                      |
| 1784                            | 21.6281                      |  | 1784                            | 25.1342                      |
| 1783                            | 21.6259                      |  | 1783                            | 25.113                       |
| 1782                            | 21.6312                      |  | 1782                            | 25.0494                      |
| 1781                            | 21.5584                      |  | 1781                            | 25.0008                      |
| 1780                            | 21.4868                      |  | 1780                            | 24.9038                      |
| 1779                            | 21.4692                      |  | 1779                            | 24.9672                      |
| 1778                            | 21.4364                      |  | 1778                            | 24.9881                      |
| 1777                            | 21.4909                      |  | 1777                            | 25.0497                      |
| 1776                            | 21.5069                      |  | 1776                            | 25.0889                      |
| 1775                            | 21.4982                      |  | 1775                            | 25.0708                      |
| 1774                            | 21.5701                      |  | 1774                            | 25.1242                      |

## FIG. 31

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1773                            | 21.6058                      |  | 1773                            | 25.1112                      |
| 1772                            | 21.6593                      |  | 1772                            | 25.1198                      |
| 1771                            | 21.6548                      |  | 1771                            | 25.04                        |
| 1770                            | 21.5662                      |  | 1770                            | 24.9756                      |
| 1769                            | 21.5506                      |  | 1769                            | 24.9833                      |
| 1768                            | 21.5329                      |  | 1768                            | 24.9787                      |
| 1767                            | 21.5638                      |  | 1767                            | 25.0205                      |
| 1766                            | 21.5737                      |  | 1766                            | 25.0414                      |
| 1765                            | 21.5358                      |  | 1765                            | 25.0413                      |
| 1764                            | 21.5528                      |  | 1764                            | 25.0751                      |
| 1763                            | 21.498                       |  | 1763                            | 25.0151                      |
| 1762                            | 21.4679                      |  | 1762                            | 25.0242                      |
| 1761                            | 21.4615                      |  | 1761                            | 25.0143                      |
| 1760                            | 21.4428                      |  | 1760                            | 25.0069                      |
| 1759                            | 21.4817                      |  | 1759                            | 25.0735                      |
| 1758                            | 21.5252                      |  | 1758                            | 25.1056                      |
| 1757                            | 21.5444                      |  | 1757                            | 25.0907                      |
| 1756                            | 21.5583                      |  | 1756                            | 25.0835                      |
| 1755                            | 21.5516                      |  | 1755                            | 25.1008                      |
| 1754                            | 21.5673                      |  | 1754                            | 25.0763                      |
| 1753                            | 21.5945                      |  | 1753                            | 25.103                       |
| 1752                            | 21.5034                      |  | 1752                            | 25.0621                      |
| 1751                            | 21.4953                      |  | 1751                            | 25.085                       |
| 1750                            | 21.4608                      |  | 1750                            | 25.0477                      |
| 1749                            | 21.4568                      |  | 1749                            | 25.0204                      |
| 1748                            | 21.5268                      |  | 1748                            | 25.0565                      |
| 1747                            | 21.5361                      |  | 1747                            | 25.0079                      |
| 1746                            | 21.5595                      |  | 1746                            | 24.9548                      |

## FIG. 32

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1745                            | 21.548                       |  | 1745                            | 24.9452                      |
| 1744                            | 21.544                       |  | 1744                            | 24.9437                      |
| 1743                            | 21.5781                      |  | 1743                            | 24.9689                      |
| 1742                            | 21.5496                      |  | 1742                            | 25.0158                      |
| 1741                            | 21.5172                      |  | 1741                            | 25.0322                      |
| 1740                            | 21.5031                      |  | 1740                            | 24.9727                      |
| 1739                            | 21.4512                      |  | 1739                            | 24.9416                      |
| 1738                            | 21.4167                      |  | 1738                            | 24.9829                      |
| 1737                            | 21.3937                      |  | 1737                            | 24.9437                      |
| 1736                            | 21.3687                      |  | 1736                            | 25.0074                      |
| 1735                            | 21.3829                      |  | 1735                            | 25.0042                      |
| 1734                            | 21.4738                      |  | 1734                            | 25.0181                      |
| 1733                            | 21.4697                      |  | 1733                            | 25.0185                      |
| 1732                            | 21.4432                      |  | 1732                            | 24.977                       |
| 1731                            | 21.4252                      |  | 1731                            | 24.9877                      |
| 1730                            | 21.399                       |  | 1730                            | 24.9378                      |
| 1729                            | 21.4046                      |  | 1729                            | 24.9457                      |
| 1728                            | 21.4366                      |  | 1728                            | 24.9759                      |
| 1727                            | 21.4524                      |  | 1727                            | 24.9718                      |
| 1726                            | 21.3466                      |  | 1726                            | 24.9845                      |
| 1725                            | 21.3439                      |  | 1725                            | 24.9541                      |
| 1724                            | 21.3039                      |  | 1724                            | 24.9351                      |
| 1723                            | 21.2334                      |  | 1723                            | 24.8937                      |
| 1722                            | 21.3122                      |  | 1722                            | 24.9518                      |
| 1721                            | 21.3891                      |  | 1721                            | 24.9565                      |
| 1720                            | 21.41                        |  | 1720                            | 24.9396                      |
| 1719                            | 21.4588                      |  | 1719                            | 25.0134                      |
| 1718                            | 21.4493                      |  | 1718                            | 24.9329                      |

## FIG. 33

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1717                            | 21.3777                      |  | 1717                            | 24.9685                      |
| 1716                            | 21.3654                      |  | 1716                            | 25.0025                      |
| 1715                            | 21.3841                      |  | 1715                            | 24.9996                      |
| 1714                            | 21.3461                      |  | 1714                            | 25.0229                      |
| 1713                            | 21.3801                      |  | 1713                            | 25.0315                      |
| 1712                            | 21.3666                      |  | 1712                            | 24.9594                      |
| 1711                            | 21.343                       |  | 1711                            | 24.9212                      |
| 1710                            | 21.3892                      |  | 1710                            | 24.9402                      |
| 1709                            | 21.3709                      |  | 1709                            | 24.971                       |
| 1708                            | 21.3678                      |  | 1708                            | 24.9768                      |
| 1707                            | 21.3624                      |  | 1707                            | 24.9773                      |
| 1706                            | 21.3933                      |  | 1706                            | 24.9599                      |
| 1705                            | 21.3822                      |  | 1705                            | 24.9167                      |
| 1704                            | 21.4226                      |  | 1704                            | 24.9873                      |
| 1703                            | 21.4438                      |  | 1703                            | 24.9836                      |
| 1702                            | 21.4248                      |  | 1702                            | 24.9446                      |
| 1701                            | 21.4083                      |  | 1701                            | 24.9482                      |
| 1700                            | 21.4082                      |  | 1700                            | 24.936                       |
| 1699                            | 21.4503                      |  | 1699                            | 24.9891                      |
| 1698                            | 21.4727                      |  | 1698                            | 25.0849                      |
| 1697                            | 21.5138                      |  | 1697                            | 25.0455                      |
| 1696                            | 21.5269                      |  | 1696                            | 25.0267                      |
| 1695                            | 21.5255                      |  | 1695                            | 25.0657                      |
| 1694                            | 21.4569                      |  | 1694                            | 24.9946                      |
| 1693                            | 21.4173                      |  | 1693                            | 24.9993                      |
| 1692                            | 21.4825                      |  | 1692                            | 25.0432                      |
| 1691                            | 21.482                       |  | 1691                            | 24.9753                      |
| 1690                            | 21.5421                      |  | 1690                            | 24.9761                      |

## FIG. 34

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1689                            | 21.5864                      |  | 1689                            | 25.0317                      |
| 1688                            | 21.5136                      |  | 1688                            | 25.0425                      |
| 1687                            | 21.5025                      |  | 1687                            | 25.0822                      |
| 1686                            | 21.4839                      |  | 1686                            | 25.0989                      |
| 1685                            | 21.5021                      |  | 1685                            | 25.0826                      |
| 1684                            | 21.5173                      |  | 1684                            | 25.0453                      |
| 1683                            | 21.5337                      |  | 1683                            | 25.0077                      |
| 1682                            | 21.5313                      |  | 1682                            | 25.0094                      |
| 1681                            | 21.5306                      |  | 1681                            | 25.0221                      |
| 1680                            | 21.5323                      |  | 1680                            | 25.0562                      |
| 1679                            | 21.4511                      |  | 1679                            | 25.0481                      |
| 1678                            | 21.4604                      |  | 1678                            | 25.029                       |
| 1677                            | 21.4186                      |  | 1677                            | 24.9907                      |
| 1676                            | 21.3868                      |  | 1676                            | 24.9569                      |
| 1675                            | 21.4639                      |  | 1675                            | 25.0073                      |
| 1674                            | 21.4881                      |  | 1674                            | 25.0483                      |
| 1673                            | 21.5227                      |  | 1673                            | 25.0905                      |
| 1672                            | 21.5122                      |  | 1672                            | 25.0409                      |
| 1671                            | 21.4362                      |  | 1671                            | 24.9785                      |
| 1670                            | 21.3969                      |  | 1670                            | 24.9686                      |
| 1669                            | 21.4185                      |  | 1669                            | 25.0333                      |
| 1668                            | 21.4329                      |  | 1668                            | 25.0735                      |
| 1667                            | 21.4691                      |  | 1667                            | 25.0755                      |
| 1666                            | 21.4841                      |  | 1666                            | 25.0521                      |
| 1665                            | 21.4642                      |  | 1665                            | 25.0251                      |
| 1664                            | 21.4871                      |  | 1664                            | 25.0824                      |
| 1663                            | 21.5143                      |  | 1663                            | 25.0971                      |
| 1662                            | 21.5215                      |  | 1662                            | 25.1366                      |

## FIG. 35

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1661                            | 21.542                       |  | 1661                            | 25.1016                      |
| 1660                            | 21.5579                      |  | 1660                            | 25.0665                      |
| 1659                            | 21.5004                      |  | 1659                            | 25.0593                      |
| 1658                            | 21.4443                      |  | 1658                            | 25.0323                      |
| 1657                            | 21.4431                      |  | 1657                            | 25.0011                      |
| 1656                            | 21.4056                      |  | 1656                            | 24.975                       |
| 1655                            | 21.4855                      |  | 1655                            | 25.0206                      |
| 1654                            | 21.4896                      |  | 1654                            | 25.0343                      |
| 1653                            | 21.4309                      |  | 1653                            | 25.0334                      |
| 1652                            | 21.4212                      |  | 1652                            | 25.0003                      |
| 1651                            | 21.409                       |  | 1651                            | 25.0117                      |
| 1650                            | 21.4512                      |  | 1650                            | 24.981                       |
| 1649                            | 21.4512                      |  | 1649                            | 24.9707                      |
| 1648                            | 21.445                       |  | 1648                            | 25.0022                      |
| 1647                            | 21.4106                      |  | 1647                            | 24.9284                      |
| 1646                            | 21.4475                      |  | 1646                            | 24.9811                      |
| 1645                            | 21.4456                      |  | 1645                            | 25.0156                      |
| 1644                            | 21.5086                      |  | 1644                            | 25.053                       |
| 1643                            | 21.5434                      |  | 1643                            | 25.1179                      |
| 1642                            | 21.509                       |  | 1642                            | 25.0157                      |
| 1641                            | 21.5234                      |  | 1641                            | 24.989                       |
| 1640                            | 21.5217                      |  | 1640                            | 24.9714                      |
| 1639                            | 21.5011                      |  | 1639                            | 24.9152                      |
| 1638                            | 21.4449                      |  | 1638                            | 24.9777                      |
| 1637                            | 21.4685                      |  | 1637                            | 25.005                       |
| 1636                            | 21.468                       |  | 1636                            | 25.027                       |
| 1635                            | 21.4637                      |  | 1635                            | 25.0628                      |
| 1634                            | 21.5137                      |  | 1634                            | 25.0576                      |

## FIG. 36

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1633                            | 21.4776                      |  | 1633                            | 25.0669                      |
| 1632                            | 21.4183                      |  | 1632                            | 25.0408                      |
| 1631                            | 21.4423                      |  | 1631                            | 25.0489                      |
| 1630                            | 21.4464                      |  | 1630                            | 25.0482                      |
| 1629                            | 21.5037                      |  | 1629                            | 25.0512                      |
| 1628                            | 21.5103                      |  | 1628                            | 25.0352                      |
| 1627                            | 21.5169                      |  | 1627                            | 25.0683                      |
| 1626                            | 21.5616                      |  | 1626                            | 25.1372                      |
| 1625                            | 21.5148                      |  | 1625                            | 25.0855                      |
| 1624                            | 21.4918                      |  | 1624                            | 25.1174                      |
| 1623                            | 21.4264                      |  | 1623                            | 25.0601                      |
| 1622                            | 21.3572                      |  | 1622                            | 25.0099                      |
| 1621                            | 21.3752                      |  | 1621                            | 25.0461                      |
| 1620                            | 21.4278                      |  | 1620                            | 25.0288                      |
| 1619                            | 21.4618                      |  | 1619                            | 25.0322                      |
| 1618                            | 21.4928                      |  | 1618                            | 25.0306                      |
| 1617                            | 21.5163                      |  | 1617                            | 25.051                       |
| 1616                            | 21.5052                      |  | 1616                            | 25.052                       |
| 1615                            | 21.4938                      |  | 1615                            | 25.0539                      |
| 1614                            | 21.4616                      |  | 1614                            | 25.0489                      |
| 1613                            | 21.433                       |  | 1613                            | 25.0295                      |
| 1612                            | 21.4221                      |  | 1612                            | 25.0475                      |
| 1611                            | 21.4406                      |  | 1611                            | 25.0623                      |
| 1610                            | 21.4593                      |  | 1610                            | 25.0136                      |
| 1609                            | 21.4785                      |  | 1609                            | 25.0324                      |
| 1608                            | 21.466                       |  | 1608                            | 24.994                       |
| 1607                            | 21.5115                      |  | 1607                            | 25.0144                      |
| 1606                            | 21.5317                      |  | 1606                            | 25.0678                      |

## FIG. 37

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1605                            | 21.5545                      |  | 1605                            | 25.0949                      |
| 1604                            | 21.597                       |  | 1604                            | 25.1263                      |
| 1603                            | 21.5148                      |  | 1603                            | 25.0577                      |
| 1602                            | 21.4856                      |  | 1602                            | 25.0189                      |
| 1601                            | 21.4853                      |  | 1601                            | 24.9799                      |
| 1600                            | 21.4519                      |  | 1600                            | 24.9666                      |
| 1599                            | 21.5169                      |  | 1599                            | 25.0494                      |
| 1598                            | 21.5601                      |  | 1598                            | 25.1015                      |
| 1597                            | 21.5258                      |  | 1597                            | 25.1221                      |
| 1596                            | 21.5351                      |  | 1596                            | 25.1217                      |
| 1595                            | 21.4795                      |  | 1595                            | 25.0497                      |
| 1594                            | 21.5093                      |  | 1594                            | 25.0629                      |
| 1593                            | 21.5491                      |  | 1593                            | 25.0753                      |
| 1592                            | 21.5914                      |  | 1592                            | 25.101                       |
| 1591                            | 21.6473                      |  | 1591                            | 25.1495                      |
| 1590                            | 21.614                       |  | 1590                            | 25.1318                      |
| 1589                            | 21.5989                      |  | 1589                            | 25.1133                      |
| 1588                            | 21.5668                      |  | 1588                            | 25.1386                      |
| 1587                            | 21.542                       |  | 1587                            | 25.1111                      |
| 1586                            | 21.5301                      |  | 1586                            | 25.0914                      |
| 1585                            | 21.5215                      |  | 1585                            | 25.0827                      |
| 1584                            | 21.5215                      |  | 1584                            | 25.0809                      |
| 1583                            | 21.5553                      |  | 1583                            | 25.1197                      |
| 1582                            | 21.5546                      |  | 1582                            | 25.1702                      |
| 1581                            | 21.5276                      |  | 1581                            | 25.1327                      |
| 1580                            | 21.5637                      |  | 1580                            | 25.1193                      |
| 1579                            | 21.5391                      |  | 1579                            | 25.0703                      |
| 1578                            | 21.5386                      |  | 1578                            | 25.0398                      |

## FIG. 38

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1577                            | 21.5653                      |  | 1577                            | 25.1162                      |
| 1576                            | 21.54                        |  | 1576                            | 25.1298                      |
| 1575                            | 21.538                       |  | 1575                            | 25.1695                      |
| 1574                            | 21.5504                      |  | 1574                            | 25.1519                      |
| 1573                            | 21.565                       |  | 1573                            | 25.1401                      |
| 1572                            | 21.5346                      |  | 1572                            | 25.089                       |
| 1571                            | 21.5624                      |  | 1571                            | 25.0729                      |
| 1570                            | 21.5613                      |  | 1570                            | 25.1165                      |
| 1569                            | 21.5191                      |  | 1569                            | 25.1151                      |
| 1568                            | 21.5572                      |  | 1568                            | 25.1614                      |
| 1567                            | 21.5344                      |  | 1567                            | 25.1848                      |
| 1566                            | 21.5428                      |  | 1566                            | 25.1556                      |
| 1565                            | 21.5685                      |  | 1565                            | 25.1467                      |
| 1564                            | 21.5738                      |  | 1564                            | 25.1497                      |
| 1563                            | 21.5643                      |  | 1563                            | 25.1017                      |
| 1562                            | 21.5443                      |  | 1562                            | 25.0984                      |
| 1561                            | 21.5445                      |  | 1561                            | 25.0743                      |
| 1560                            | 21.5938                      |  | 1560                            | 25.097                       |
| 1559                            | 21.6258                      |  | 1559                            | 25.1118                      |
| 1558                            | 21.6628                      |  | 1558                            | 25.1253                      |
| 1557                            | 21.7105                      |  | 1557                            | 25.1511                      |
| 1556                            | 21.6129                      |  | 1556                            | 25.0779                      |
| 1555                            | 21.5916                      |  | 1555                            | 25.0726                      |
| 1554                            | 21.6051                      |  | 1554                            | 25.0935                      |
| 1553                            | 21.5529                      |  | 1553                            | 25.0508                      |
| 1552                            | 21.6116                      |  | 1552                            | 25.1257                      |
| 1551                            | 21.6027                      |  | 1551                            | 25.1503                      |
| 1550                            | 21.5542                      |  | 1550                            | 25.1206                      |

## FIG. 39

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1549                            | 21.5795                      |  | 1549                            | 25.1563                      |
| 1548                            | 21.5992                      |  | 1548                            | 25.1214                      |
| 1547                            | 21.5992                      |  | 1547                            | 25.1463                      |
| 1546                            | 21.5807                      |  | 1546                            | 25.1491                      |
| 1545                            | 21.5544                      |  | 1545                            | 25.1056                      |
| 1544                            | 21.5345                      |  | 1544                            | 25.0916                      |
| 1543                            | 21.5559                      |  | 1543                            | 25.0597                      |
| 1542                            | 21.5783                      |  | 1542                            | 25.0598                      |
| 1541                            | 21.6157                      |  | 1541                            | 25.1236                      |
| 1540                            | 21.6484                      |  | 1540                            | 25.1574                      |
| 1539                            | 21.6418                      |  | 1539                            | 25.1711                      |
| 1538                            | 21.6625                      |  | 1538                            | 25.1968                      |
| 1537                            | 21.6335                      |  | 1537                            | 25.1926                      |
| 1536                            | 21.5672                      |  | 1536                            | 25.1451                      |
| 1535                            | 21.5801                      |  | 1535                            | 25.1673                      |
| 1534                            | 21.5361                      |  | 1534                            | 25.1114                      |
| 1533                            | 21.5136                      |  | 1533                            | 25.0937                      |
| 1532                            | 21.5609                      |  | 1532                            | 25.1297                      |
| 1531                            | 21.5364                      |  | 1531                            | 25.0728                      |
| 1530                            | 21.542                       |  | 1530                            | 25.1084                      |
| 1529                            | 21.5721                      |  | 1529                            | 25.1221                      |
| 1528                            | 21.5337                      |  | 1528                            | 25.1204                      |
| 1527                            | 21.5186                      |  | 1527                            | 25.1398                      |
| 1526                            | 21.5321                      |  | 1526                            | 25.1203                      |
| 1525                            | 21.5322                      |  | 1525                            | 25.1145                      |
| 1524                            | 21.5521                      |  | 1524                            | 25.0973                      |
| 1523                            | 21.554                       |  | 1523                            | 25.0857                      |
| 1522                            | 21.5823                      |  | 1522                            | 25.1341                      |

## FIG. 40

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1521                            | 21.5829                      |  | 1521                            | 25.1041                      |
| 1520                            | 21.5642                      |  | 1520                            | 25.0825                      |
| 1519                            | 21.5752                      |  | 1519                            | 25.081                       |
| 1518                            | 21.5353                      |  | 1518                            | 25.0221                      |
| 1517                            | 21.5531                      |  | 1517                            | 25.0171                      |
| 1516                            | 21.5222                      |  | 1516                            | 25.0482                      |
| 1515                            | 21.5524                      |  | 1515                            | 25.066                       |
| 1514                            | 21.5702                      |  | 1514                            | 25.0851                      |
| 1513                            | 21.566                       |  | 1513                            | 25.1168                      |
| 1512                            | 21.5691                      |  | 1512                            | 25.1047                      |
| 1511                            | 21.5376                      |  | 1511                            | 25.0909                      |
| 1510                            | 21.5092                      |  | 1510                            | 25.0571                      |
| 1509                            | 21.4905                      |  | 1509                            | 25.0554                      |
| 1508                            | 21.5092                      |  | 1508                            | 25.0605                      |
| 1507                            | 21.5166                      |  | 1507                            | 25.0474                      |
| 1506                            | 21.5408                      |  | 1506                            | 25.0868                      |
| 1505                            | 21.5356                      |  | 1505                            | 25.078                       |
| 1504                            | 21.5051                      |  | 1504                            | 25.0639                      |
| 1503                            | 21.5158                      |  | 1503                            | 25.0906                      |
| 1502                            | 21.5406                      |  | 1502                            | 25.0994                      |
| 1501                            | 21.5623                      |  | 1501                            | 25.0739                      |
| 1500                            | 21.5804                      |  | 1500                            | 25.0524                      |
| 1499                            | 21.628                       |  | 1499                            | 25.0347                      |
| 1498                            | 21.5901                      |  | 1498                            | 24.9892                      |
| 1497                            | 21.5682                      |  | 1497                            | 25.0125                      |
| 1496                            | 21.5784                      |  | 1496                            | 25.0229                      |
| 1495                            | 21.5329                      |  | 1495                            | 25.044                       |
| 1494                            | 21.5779                      |  | 1494                            | 25.0695                      |

## FIG. 41

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1493                            | 21.5748                      |  | 1493                            | 25.0489                      |
| 1492                            | 21.6102                      |  | 1492                            | 25.0822                      |
| 1491                            | 21.5803                      |  | 1491                            | 25.0799                      |
| 1490                            | 21.5626                      |  | 1490                            | 25.0924                      |
| 1489                            | 21.5463                      |  | 1489                            | 25.1028                      |
| 1488                            | 21.5306                      |  | 1488                            | 25.0816                      |
| 1487                            | 21.5599                      |  | 1487                            | 25.085                       |
| 1486                            | 21.5352                      |  | 1486                            | 25.0865                      |
| 1485                            | 21.5345                      |  | 1485                            | 25.0718                      |
| 1484                            | 21.5295                      |  | 1484                            | 25.0749                      |
| 1483                            | 21.5198                      |  | 1483                            | 25.0421                      |
| 1482                            | 21.5595                      |  | 1482                            | 25.0355                      |
| 1481                            | 21.5738                      |  | 1481                            | 25.0815                      |
| 1480                            | 21.5841                      |  | 1480                            | 25.076                       |
| 1479                            | 21.6107                      |  | 1479                            | 25.1384                      |
| 1478                            | 21.5496                      |  | 1478                            | 25.099                       |
| 1477                            | 21.5587                      |  | 1477                            | 25.0728                      |
| 1476                            | 21.5564                      |  | 1476                            | 25.1121                      |
| 1475                            | 21.4926                      |  | 1475                            | 25.0596                      |
| 1474                            | 21.5133                      |  | 1474                            | 25.074                       |
| 1473                            | 21.5002                      |  | 1473                            | 25.0474                      |
| 1472                            | 21.5163                      |  | 1472                            | 25.0181                      |
| 1471                            | 21.5579                      |  | 1471                            | 25.0429                      |
| 1470                            | 21.5505                      |  | 1470                            | 25.0589                      |
| 1469                            | 21.5499                      |  | 1469                            | 25.0806                      |
| 1468                            | 21.4888                      |  | 1468                            | 25.0576                      |
| 1467                            | 21.4567                      |  | 1467                            | 25.0177                      |
| 1466                            | 21.445                       |  | 1466                            | 25.0132                      |

## FIG. 42

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1465                            | 21.455                       |  | 1465                            | 25.0211                      |
| 1464                            | 21.503                       |  | 1464                            | 25.0559                      |
| 1463                            | 21.5428                      |  | 1463                            | 25.0609                      |
| 1462                            | 21.5687                      |  | 1462                            | 25.0711                      |
| 1461                            | 21.5427                      |  | 1461                            | 25.0516                      |
| 1460                            | 21.526                       |  | 1460                            | 25.0412                      |
| 1459                            | 21.5279                      |  | 1459                            | 25.0495                      |
| 1458                            | 21.5194                      |  | 1458                            | 25.0428                      |
| 1457                            | 21.5227                      |  | 1457                            | 25.0455                      |
| 1456                            | 21.5401                      |  | 1456                            | 25.0552                      |
| 1455                            | 21.4974                      |  | 1455                            | 25.0203                      |
| 1454                            | 21.54                        |  | 1454                            | 25.024                       |
| 1453                            | 21.5516                      |  | 1453                            | 25.031                       |
| 1452                            | 21.525                       |  | 1452                            | 25.0156                      |
| 1451                            | 21.5291                      |  | 1451                            | 25.0521                      |
| 1450                            | 21.4738                      |  | 1450                            | 25.0526                      |
| 1449                            | 21.4876                      |  | 1449                            | 25.0726                      |
| 1448                            | 21.4757                      |  | 1448                            | 25.0577                      |
| 1447                            | 21.463                       |  | 1447                            | 25.0525                      |
| 1446                            | 21.5172                      |  | 1446                            | 25.0524                      |
| 1445                            | 21.4951                      |  | 1445                            | 25.0344                      |
| 1444                            | 21.534                       |  | 1444                            | 25.018                       |
| 1443                            | 21.5605                      |  | 1443                            | 25.0127                      |
| 1442                            | 21.5087                      |  | 1442                            | 25.0094                      |
| 1441                            | 21.4903                      |  | 1441                            | 24.9761                      |
| 1440                            | 21.4877                      |  | 1440                            | 24.9793                      |
| 1439                            | 21.4333                      |  | 1439                            | 25.0039                      |
| 1438                            | 21.5059                      |  | 1438                            | 25.0186                      |

## FIG. 43

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1437                            | 21.529                       |  | 1437                            | 25.0311                      |
| 1436                            | 21.5424                      |  | 1436                            | 25.0425                      |
| 1435                            | 21.5606                      |  | 1435                            | 25.0481                      |
| 1434                            | 21.4657                      |  | 1434                            | 24.9908                      |
| 1433                            | 21.4464                      |  | 1433                            | 25.0139                      |
| 1432                            | 21.4498                      |  | 1432                            | 25.0187                      |
| 1431                            | 21.4302                      |  | 1431                            | 24.9958                      |
| 1430                            | 21.4816                      |  | 1430                            | 25.0384                      |
| 1429                            | 21.4825                      |  | 1429                            | 25.0511                      |
| 1428                            | 21.4847                      |  | 1428                            | 25.0324                      |
| 1427                            | 21.4977                      |  | 1427                            | 25.0408                      |
| 1426                            | 21.479                       |  | 1426                            | 25.0197                      |
| 1425                            | 21.5028                      |  | 1425                            | 25.0467                      |
| 1424                            | 21.4996                      |  | 1424                            | 25.0448                      |
| 1423                            | 21.4928                      |  | 1423                            | 25.0282                      |
| 1422                            | 21.5322                      |  | 1422                            | 25.0548                      |
| 1421                            | 21.5182                      |  | 1421                            | 25.0132                      |
| 1420                            | 21.5279                      |  | 1420                            | 25.0264                      |
| 1419                            | 21.5299                      |  | 1419                            | 25.0461                      |
| 1418                            | 21.5222                      |  | 1418                            | 25.041                       |
| 1417                            | 21.5615                      |  | 1417                            | 25.049                       |
| 1416                            | 21.5919                      |  | 1416                            | 25.0818                      |
| 1415                            | 21.592                       |  | 1415                            | 25.0698                      |
| 1414                            | 21.6213                      |  | 1414                            | 25.0711                      |
| 1413                            | 21.6084                      |  | 1413                            | 25.0755                      |
| 1412                            | 21.5935                      |  | 1412                            | 25.0614                      |
| 1411                            | 21.6131                      |  | 1411                            | 25.0829                      |
| 1410                            | 21.5737                      |  | 1410                            | 25.0876                      |

**FIG. 44**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1409                            | 21.6005                      |  | 1409                            | 25.0893                      |
| 1408                            | 21.6061                      |  | 1408                            | 25.125                       |
| 1407                            | 21.5951                      |  | 1407                            | 25.1227                      |
| 1406                            | 21.5882                      |  | 1406                            | 25.1334                      |
| 1405                            | 21.5776                      |  | 1405                            | 25.1592                      |
| 1404                            | 21.5904                      |  | 1404                            | 25.1558                      |
| 1403                            | 21.6017                      |  | 1403                            | 25.1742                      |
| 1402                            | 21.6435                      |  | 1402                            | 25.1903                      |
| 1401                            | 21.6315                      |  | 1401                            | 25.1666                      |
| 1400                            | 21.5982                      |  | 1400                            | 25.1478                      |
| 1399                            | 21.5928                      |  | 1399                            | 25.1054                      |
| 1398                            | 21.5569                      |  | 1398                            | 25.0789                      |
| 1397                            | 21.5525                      |  | 1397                            | 25.0811                      |
| 1396                            | 21.5808                      |  | 1396                            | 25.0859                      |
| 1395                            | 21.5739                      |  | 1395                            | 25.0989                      |
| 1394                            | 21.6037                      |  | 1394                            | 25.1153                      |
| 1393                            | 21.6274                      |  | 1393                            | 25.1332                      |
| 1392                            | 21.6214                      |  | 1392                            | 25.1318                      |
| 1391                            | 21.6397                      |  | 1391                            | 25.138                       |
| 1390                            | 21.6307                      |  | 1390                            | 25.1302                      |
| 1389                            | 21.6193                      |  | 1389                            | 25.1124                      |
| 1388                            | 21.6213                      |  | 1388                            | 25.1116                      |
| 1387                            | 21.5947                      |  | 1387                            | 25.135                       |
| 1386                            | 21.6102                      |  | 1386                            | 25.1562                      |
| 1385                            | 21.6373                      |  | 1385                            | 25.1863                      |
| 1384                            | 21.6353                      |  | 1384                            | 25.1994                      |
| 1383                            | 21.6734                      |  | 1383                            | 25.2154                      |
| 1382                            | 21.6609                      |  | 1382                            | 25.2227                      |

## FIG. 45

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1381                            | 21.6783                      |  | 1381                            | 25.2145                      |
| 1380                            | 21.7003                      |  | 1380                            | 25.2359                      |
| 1379                            | 21.6928                      |  | 1379                            | 25.2061                      |
| 1378                            | 21.7086                      |  | 1378                            | 25.2249                      |
| 1377                            | 21.6623                      |  | 1377                            | 25.2306                      |
| 1376                            | 21.6632                      |  | 1376                            | 25.2287                      |
| 1375                            | 21.6922                      |  | 1375                            | 25.2726                      |
| 1374                            | 21.6866                      |  | 1374                            | 25.2354                      |
| 1373                            | 21.6948                      |  | 1373                            | 25.2275                      |
| 1372                            | 21.7095                      |  | 1372                            | 25.2699                      |
| 1371                            | 21.6939                      |  | 1371                            | 25.2802                      |
| 1370                            | 21.7195                      |  | 1370                            | 25.3332                      |
| 1369                            | 21.7608                      |  | 1369                            | 25.3521                      |
| 1368                            | 21.7347                      |  | 1368                            | 25.3169                      |
| 1367                            | 21.7501                      |  | 1367                            | 25.3205                      |
| 1366                            | 21.7432                      |  | 1366                            | 25.3088                      |
| 1365                            | 21.7054                      |  | 1365                            | 25.3119                      |
| 1364                            | 21.7485                      |  | 1364                            | 25.3118                      |
| 1363                            | 21.7467                      |  | 1363                            | 25.3047                      |
| 1362                            | 21.7567                      |  | 1362                            | 25.3018                      |
| 1361                            | 21.7668                      |  | 1361                            | 25.2984                      |
| 1360                            | 21.7463                      |  | 1360                            | 25.3127                      |
| 1359                            | 21.7382                      |  | 1359                            | 25.3115                      |
| 1358                            | 21.7181                      |  | 1358                            | 25.3154                      |
| 1357                            | 21.7397                      |  | 1357                            | 25.3181                      |
| 1356                            | 21.7179                      |  | 1356                            | 25.2853                      |
| 1355                            | 21.709                       |  | 1355                            | 25.265                       |
| 1354                            | 21.7143                      |  | 1354                            | 25.2553                      |

## FIG. 46

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1353                            | 21.6977                      |  | 1353                            | 25.259                       |
| 1352                            | 21.7052                      |  | 1352                            | 25.2662                      |
| 1351                            | 21.7031                      |  | 1351                            | 25.2771                      |
| 1350                            | 21.7064                      |  | 1350                            | 25.2896                      |
| 1349                            | 21.7197                      |  | 1349                            | 25.2895                      |
| 1348                            | 21.7398                      |  | 1348                            | 25.2985                      |
| 1347                            | 21.7562                      |  | 1347                            | 25.2915                      |
| 1346                            | 21.7474                      |  | 1346                            | 25.2771                      |
| 1345                            | 21.7494                      |  | 1345                            | 25.2754                      |
| 1344                            | 21.7386                      |  | 1344                            | 25.2652                      |
| 1343                            | 21.7322                      |  | 1343                            | 25.28                        |
| 1342                            | 21.7532                      |  | 1342                            | 25.2886                      |
| 1341                            | 21.7196                      |  | 1341                            | 25.2857                      |
| 1340                            | 21.7043                      |  | 1340                            | 25.2886                      |
| 1339                            | 21.6898                      |  | 1339                            | 25.2834                      |
| 1338                            | 21.6555                      |  | 1338                            | 25.2528                      |
| 1337                            | 21.6799                      |  | 1337                            | 25.2458                      |
| 1336                            | 21.6912                      |  | 1336                            | 25.2606                      |
| 1335                            | 21.7226                      |  | 1335                            | 25.2636                      |
| 1334                            | 21.7489                      |  | 1334                            | 25.2737                      |
| 1333                            | 21.7518                      |  | 1333                            | 25.258                       |
| 1332                            | 21.7527                      |  | 1332                            | 25.2214                      |
| 1331                            | 21.7296                      |  | 1331                            | 25.2148                      |
| 1330                            | 21.7259                      |  | 1330                            | 25.2304                      |
| 1329                            | 21.7086                      |  | 1329                            | 25.2489                      |
| 1328                            | 21.7121                      |  | 1328                            | 25.2723                      |
| 1327                            | 21.6991                      |  | 1327                            | 25.2566                      |
| 1326                            | 21.6719                      |  | 1326                            | 25.2483                      |

**FIG. 47**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1325                            | 21.6906                      |  | 1325                            | 25.2494                      |
| 1324                            | 21.7019                      |  | 1324                            | 25.2371                      |
| 1323                            | 21.705                       |  | 1323                            | 25.2142                      |
| 1322                            | 21.7234                      |  | 1322                            | 25.1828                      |
| 1321                            | 21.7117                      |  | 1321                            | 25.1611                      |
| 1320                            | 21.6893                      |  | 1320                            | 25.1596                      |
| 1319                            | 21.6969                      |  | 1319                            | 25.1989                      |
| 1318                            | 21.7038                      |  | 1318                            | 25.2298                      |
| 1317                            | 21.6844                      |  | 1317                            | 25.2415                      |
| 1316                            | 21.6985                      |  | 1316                            | 25.2321                      |
| 1315                            | 21.6836                      |  | 1315                            | 25.2119                      |
| 1314                            | 21.6583                      |  | 1314                            | 25.1853                      |
| 1313                            | 21.6631                      |  | 1313                            | 25.174                       |
| 1312                            | 21.6542                      |  | 1312                            | 25.1855                      |
| 1311                            | 21.6635                      |  | 1311                            | 25.1785                      |
| 1310                            | 21.6729                      |  | 1310                            | 25.1972                      |
| 1309                            | 21.6697                      |  | 1309                            | 25.185                       |
| 1308                            | 21.6533                      |  | 1308                            | 25.1755                      |
| 1307                            | 21.6464                      |  | 1307                            | 25.171                       |
| 1306                            | 21.6302                      |  | 1306                            | 25.1488                      |
| 1305                            | 21.66                        |  | 1305                            | 25.1778                      |
| 1304                            | 21.659                       |  | 1304                            | 25.1803                      |
| 1303                            | 21.6747                      |  | 1303                            | 25.2062                      |
| 1302                            | 21.6849                      |  | 1302                            | 25.1953                      |
| 1301                            | 21.666                       |  | 1301                            | 25.1792                      |
| 1300                            | 21.6936                      |  | 1300                            | 25.1739                      |
| 1299                            | 21.6685                      |  | 1299                            | 25.1673                      |
| 1298                            | 21.6731                      |  | 1298                            | 25.1782                      |

**FIG. 48**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1297                            | 21.6505                      |  | 1297                            | 25.1482                      |
| 1296                            | 21.6388                      |  | 1296                            | 25.1527                      |
| 1295                            | 21.6548                      |  | 1295                            | 25.1294                      |
| 1294                            | 21.656                       |  | 1294                            | 25.1232                      |
| 1293                            | 21.6518                      |  | 1293                            | 25.13                        |
| 1292                            | 21.6396                      |  | 1292                            | 25.1404                      |
| 1291                            | 21.623                       |  | 1291                            | 25.1539                      |
| 1290                            | 21.6283                      |  | 1290                            | 25.1749                      |
| 1289                            | 21.6272                      |  | 1289                            | 25.1664                      |
| 1288                            | 21.618                       |  | 1288                            | 25.1493                      |
| 1287                            | 21.6256                      |  | 1287                            | 25.1406                      |
| 1286                            | 21.6192                      |  | 1286                            | 25.1363                      |
| 1285                            | 21.6303                      |  | 1285                            | 25.1599                      |
| 1284                            | 21.6298                      |  | 1284                            | 25.1561                      |
| 1283                            | 21.6384                      |  | 1283                            | 25.1558                      |
| 1282                            | 21.6303                      |  | 1282                            | 25.15                        |
| 1281                            | 21.6529                      |  | 1281                            | 25.1425                      |
| 1280                            | 21.6644                      |  | 1280                            | 25.1496                      |
| 1279                            | 21.6422                      |  | 1279                            | 25.1568                      |
| 1278                            | 21.6397                      |  | 1278                            | 25.1343                      |
| 1277                            | 21.6224                      |  | 1277                            | 25.1288                      |
| 1276                            | 21.5941                      |  | 1276                            | 25.0972                      |
| 1275                            | 21.6056                      |  | 1275                            | 25.0904                      |
| 1274                            | 21.6172                      |  | 1274                            | 25.1165                      |
| 1273                            | 21.6212                      |  | 1273                            | 25.1158                      |
| 1272                            | 21.6569                      |  | 1272                            | 25.1532                      |
| 1271                            | 21.6462                      |  | 1271                            | 25.1312                      |
| 1270                            | 21.6296                      |  | 1270                            | 25.1032                      |

## FIG. 49

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1269                            | 21.6239                      |  | 1269                            | 25.1122                      |
| 1268                            | 21.6119                      |  | 1268                            | 25.1116                      |
| 1267                            | 21.6224                      |  | 1267                            | 25.1175                      |
| 1266                            | 21.614                       |  | 1266                            | 25.1174                      |
| 1265                            | 21.5989                      |  | 1265                            | 25.0947                      |
| 1264                            | 21.6034                      |  | 1264                            | 25.0698                      |
| 1263                            | 21.5881                      |  | 1263                            | 25.0748                      |
| 1262                            | 21.595                       |  | 1262                            | 25.0729                      |
| 1261                            | 21.604                       |  | 1261                            | 25.0867                      |
| 1260                            | 21.6041                      |  | 1260                            | 25.0813                      |
| 1259                            | 21.6246                      |  | 1259                            | 25.0897                      |
| 1258                            | 21.6257                      |  | 1258                            | 25.1007                      |
| 1257                            | 21.631                       |  | 1257                            | 25.0973                      |
| 1256                            | 21.6373                      |  | 1256                            | 25.1061                      |
| 1255                            | 21.6218                      |  | 1255                            | 25.0767                      |
| 1254                            | 21.6123                      |  | 1254                            | 25.0736                      |
| 1253                            | 21.6185                      |  | 1253                            | 25.0787                      |
| 1252                            | 21.6211                      |  | 1252                            | 25.0819                      |
| 1251                            | 21.6583                      |  | 1251                            | 25.1207                      |
| 1250                            | 21.6904                      |  | 1250                            | 25.1442                      |
| 1249                            | 21.6875                      |  | 1249                            | 25.1482                      |
| 1248                            | 21.6774                      |  | 1248                            | 25.1727                      |
| 1247                            | 21.6538                      |  | 1247                            | 25.1667                      |
| 1246                            | 21.6687                      |  | 1246                            | 25.1814                      |
| 1245                            | 21.6781                      |  | 1245                            | 25.1862                      |
| 1244                            | 21.6926                      |  | 1244                            | 25.1835                      |
| 1243                            | 21.7148                      |  | 1243                            | 25.2056                      |
| 1242                            | 21.7045                      |  | 1242                            | 25.2007                      |

## FIG. 50

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1241                            | 21.7013                      |  | 1241                            | 25.2223                      |
| 1240                            | 21.6967                      |  | 1240                            | 25.2142                      |
| 1239                            | 21.7082                      |  | 1239                            | 25.2213                      |
| 1238                            | 21.721                       |  | 1238                            | 25.2238                      |
| 1237                            | 21.7363                      |  | 1237                            | 25.2029                      |
| 1236                            | 21.7348                      |  | 1236                            | 25.2072                      |
| 1235                            | 21.7212                      |  | 1235                            | 25.1983                      |
| 1234                            | 21.7032                      |  | 1234                            | 25.2162                      |
| 1233                            | 21.6839                      |  | 1233                            | 25.2285                      |
| 1232                            | 21.6879                      |  | 1232                            | 25.2178                      |
| 1231                            | 21.6878                      |  | 1231                            | 25.2234                      |
| 1230                            | 21.6961                      |  | 1230                            | 25.2127                      |
| 1229                            | 21.6896                      |  | 1229                            | 25.2091                      |
| 1228                            | 21.6997                      |  | 1228                            | 25.2178                      |
| 1227                            | 21.7032                      |  | 1227                            | 25.197                       |
| 1226                            | 21.7139                      |  | 1226                            | 25.1829                      |
| 1225                            | 21.7387                      |  | 1225                            | 25.1873                      |
| 1224                            | 21.7094                      |  | 1224                            | 25.1797                      |
| 1223                            | 21.706                       |  | 1223                            | 25.1857                      |
| 1222                            | 21.6985                      |  | 1222                            | 25.1754                      |
| 1221                            | 21.6747                      |  | 1221                            | 25.1618                      |
| 1220                            | 21.6942                      |  | 1220                            | 25.1727                      |
| 1219                            | 21.6656                      |  | 1219                            | 25.1389                      |
| 1218                            | 21.6574                      |  | 1218                            | 25.1432                      |
| 1217                            | 21.6814                      |  | 1217                            | 25.154                       |
| 1216                            | 21.6865                      |  | 1216                            | 25.1438                      |
| 1215                            | 21.7084                      |  | 1215                            | 25.1915                      |
| 1214                            | 21.7026                      |  | 1214                            | 25.179                       |

## FIG. 51

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1213                            | 21.6916                      |  | 1213                            | 25.1608                      |
| 1212                            | 21.682                       |  | 1212                            | 25.173                       |
| 1211                            | 21.6629                      |  | 1211                            | 25.1373                      |
| 1210                            | 21.6561                      |  | 1210                            | 25.1438                      |
| 1209                            | 21.6697                      |  | 1209                            | 25.154                       |
| 1208                            | 21.6817                      |  | 1208                            | 25.1583                      |
| 1207                            | 21.6909                      |  | 1207                            | 25.1569                      |
| 1206                            | 21.7006                      |  | 1206                            | 25.1638                      |
| 1205                            | 21.6762                      |  | 1205                            | 25.1666                      |
| 1204                            | 21.6455                      |  | 1204                            | 25.1426                      |
| 1203                            | 21.6435                      |  | 1203                            | 25.1381                      |
| 1202                            | 21.6238                      |  | 1202                            | 25.1163                      |
| 1201                            | 21.6216                      |  | 1201                            | 25.089                       |
| 1200                            | 21.6087                      |  | 1200                            | 25.1216                      |
| 1199                            | 21.5938                      |  | 1199                            | 25.1169                      |
| 1198                            | 21.5977                      |  | 1198                            | 25.1288                      |
| 1197                            | 21.6052                      |  | 1197                            | 25.1373                      |
| 1196                            | 21.6131                      |  | 1196                            | 25.1312                      |
| 1195                            | 21.6098                      |  | 1195                            | 25.1255                      |
| 1194                            | 21.627                       |  | 1194                            | 25.1425                      |
| 1193                            | 21.629                       |  | 1193                            | 25.1141                      |
| 1192                            | 21.6394                      |  | 1192                            | 25.1178                      |
| 1191                            | 21.6438                      |  | 1191                            | 25.1302                      |
| 1190                            | 21.6387                      |  | 1190                            | 25.1144                      |
| 1189                            | 21.6292                      |  | 1189                            | 25.1314                      |
| 1188                            | 21.6234                      |  | 1188                            | 25.1297                      |
| 1187                            | 21.6403                      |  | 1187                            | 25.1318                      |
| 1186                            | 21.6337                      |  | 1186                            | 25.1291                      |

## FIG. 52

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1185                            | 21.6285                      |  | 1185                            | 25.1137                      |
| 1184                            | 21.6093                      |  | 1184                            | 25.0976                      |
| 1183                            | 21.595                       |  | 1183                            | 25.0905                      |
| 1182                            | 21.5918                      |  | 1182                            | 25.0922                      |
| 1181                            | 21.6065                      |  | 1181                            | 25.1132                      |
| 1180                            | 21.6299                      |  | 1180                            | 25.1325                      |
| 1179                            | 21.6563                      |  | 1179                            | 25.128                       |
| 1178                            | 21.6701                      |  | 1178                            | 25.1272                      |
| 1177                            | 21.665                       |  | 1177                            | 25.1203                      |
| 1176                            | 21.6362                      |  | 1176                            | 25.1055                      |
| 1175                            | 21.613                       |  | 1175                            | 25.1119                      |
| 1174                            | 21.61                        |  | 1174                            | 25.1181                      |
| 1173                            | 21.6429                      |  | 1173                            | 25.1362                      |
| 1172                            | 21.6733                      |  | 1172                            | 25.1538                      |
| 1171                            | 21.672                       |  | 1171                            | 25.1439                      |
| 1170                            | 21.6867                      |  | 1170                            | 25.15                        |
| 1169                            | 21.638                       |  | 1169                            | 25.1177                      |
| 1168                            | 21.6377                      |  | 1168                            | 25.1158                      |
| 1167                            | 21.6412                      |  | 1167                            | 25.1223                      |
| 1166                            | 21.6335                      |  | 1166                            | 25.1227                      |
| 1165                            | 21.6519                      |  | 1165                            | 25.1231                      |
| 1164                            | 21.6377                      |  | 1164                            | 25.1084                      |
| 1163                            | 21.6445                      |  | 1163                            | 25.1142                      |
| 1162                            | 21.6236                      |  | 1162                            | 25.1064                      |
| 1161                            | 21.6068                      |  | 1161                            | 25.0972                      |
| 1160                            | 21.617                       |  | 1160                            | 25.0945                      |
| 1159                            | 21.6098                      |  | 1159                            | 25.1023                      |
| 1158                            | 21.6067                      |  | 1158                            | 25.0942                      |

## FIG. 53

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1157                            | 21.6263                      |  | 1157                            | 25.1059                      |
| 1156                            | 21.63                        |  | 1156                            | 25.1283                      |
| 1155                            | 21.6358                      |  | 1155                            | 25.1174                      |
| 1154                            | 21.6446                      |  | 1154                            | 25.1194                      |
| 1153                            | 21.63                        |  | 1153                            | 25.1137                      |
| 1152                            | 21.6274                      |  | 1152                            | 25.1053                      |
| 1151                            | 21.6151                      |  | 1151                            | 25.1166                      |
| 1150                            | 21.6021                      |  | 1150                            | 25.114                       |
| 1149                            | 21.6082                      |  | 1149                            | 25.1121                      |
| 1148                            | 21.6035                      |  | 1148                            | 25.1124                      |
| 1147                            | 21.6072                      |  | 1147                            | 25.1101                      |
| 1146                            | 21.6103                      |  | 1146                            | 25.0942                      |
| 1145                            | 21.6164                      |  | 1145                            | 25.1016                      |
| 1144                            | 21.615                       |  | 1144                            | 25.0942                      |
| 1143                            | 21.601                       |  | 1143                            | 25.0813                      |
| 1142                            | 21.6192                      |  | 1142                            | 25.1046                      |
| 1141                            | 21.6081                      |  | 1141                            | 25.0928                      |
| 1140                            | 21.621                       |  | 1140                            | 25.1039                      |
| 1139                            | 21.6374                      |  | 1139                            | 25.1015                      |
| 1138                            | 21.632                       |  | 1138                            | 25.0915                      |
| 1137                            | 21.6438                      |  | 1137                            | 25.1066                      |
| 1136                            | 21.6226                      |  | 1136                            | 25.081                       |
| 1135                            | 21.6033                      |  | 1135                            | 25.0718                      |
| 1134                            | 21.6038                      |  | 1134                            | 25.083                       |
| 1133                            | 21.5987                      |  | 1133                            | 25.0958                      |
| 1132                            | 21.6108                      |  | 1132                            | 25.1032                      |
| 1131                            | 21.6195                      |  | 1131                            | 25.0956                      |
| 1130                            | 21.6227                      |  | 1130                            | 25.0945                      |

## FIG. 54

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1129                            | 21.6118                      |  | 1129                            | 25.0622                      |
| 1128                            | 21.6048                      |  | 1128                            | 25.0747                      |
| 1127                            | 21.6231                      |  | 1127                            | 25.0883                      |
| 1126                            | 21.6329                      |  | 1126                            | 25.0884                      |
| 1125                            | 21.6452                      |  | 1125                            | 25.1005                      |
| 1124                            | 21.644                       |  | 1124                            | 25.0851                      |
| 1123                            | 21.6268                      |  | 1123                            | 25.0826                      |
| 1122                            | 21.6137                      |  | 1122                            | 25.0758                      |
| 1121                            | 21.6266                      |  | 1121                            | 25.0828                      |
| 1120                            | 21.6389                      |  | 1120                            | 25.0947                      |
| 1119                            | 21.638                       |  | 1119                            | 25.1038                      |
| 1118                            | 21.6437                      |  | 1118                            | 25.1136                      |
| 1117                            | 21.6502                      |  | 1117                            | 25.1247                      |
| 1116                            | 21.6412                      |  | 1116                            | 25.1268                      |
| 1115                            | 21.6491                      |  | 1115                            | 25.1367                      |
| 1114                            | 21.6505                      |  | 1114                            | 25.1296                      |
| 1113                            | 21.6404                      |  | 1113                            | 25.1208                      |
| 1112                            | 21.6326                      |  | 1112                            | 25.0968                      |
| 1111                            | 21.6279                      |  | 1111                            | 25.0834                      |
| 1110                            | 21.6209                      |  | 1110                            | 25.0811                      |
| 1109                            | 21.6071                      |  | 1109                            | 25.0535                      |
| 1108                            | 21.6211                      |  | 1108                            | 25.0768                      |
| 1107                            | 21.6352                      |  | 1107                            | 25.0839                      |
| 1106                            | 21.6399                      |  | 1106                            | 25.0822                      |
| 1105                            | 21.66                        |  | 1105                            | 25.1128                      |
| 1104                            | 21.6501                      |  | 1104                            | 25.109                       |
| 1103                            | 21.6272                      |  | 1103                            | 25.092                       |
| 1102                            | 21.618                       |  | 1102                            | 25.0934                      |

## FIG. 55

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1101                            | 21.5967                      |  | 1101                            | 25.089                       |
| 1100                            | 21.6103                      |  | 1100                            | 25.0891                      |
| 1099                            | 21.6338                      |  | 1099                            | 25.1005                      |
| 1098                            | 21.628                       |  | 1098                            | 25.0901                      |
| 1097                            | 21.6222                      |  | 1097                            | 25.0675                      |
| 1096                            | 21.6129                      |  | 1096                            | 25.0525                      |
| 1095                            | 21.5903                      |  | 1095                            | 25.0376                      |
| 1094                            | 21.5842                      |  | 1094                            | 25.0274                      |
| 1093                            | 21.5766                      |  | 1093                            | 25.0258                      |
| 1092                            | 21.5804                      |  | 1092                            | 25.0359                      |
| 1091                            | 21.5943                      |  | 1091                            | 25.0435                      |
| 1090                            | 21.6172                      |  | 1090                            | 25.0599                      |
| 1089                            | 21.6337                      |  | 1089                            | 25.0793                      |
| 1088                            | 21.6424                      |  | 1088                            | 25.0822                      |
| 1087                            | 21.6363                      |  | 1087                            | 25.0858                      |
| 1086                            | 21.6419                      |  | 1086                            | 25.0852                      |
| 1085                            | 21.6347                      |  | 1085                            | 25.0779                      |
| 1084                            | 21.621                       |  | 1084                            | 25.0735                      |
| 1083                            | 21.6097                      |  | 1083                            | 25.0604                      |
| 1082                            | 21.6075                      |  | 1082                            | 25.0609                      |
| 1081                            | 21.6124                      |  | 1081                            | 25.0713                      |
| 1080                            | 21.6092                      |  | 1080                            | 25.0762                      |
| 1079                            | 21.633                       |  | 1079                            | 25.085                       |
| 1078                            | 21.6296                      |  | 1078                            | 25.0753                      |
| 1077                            | 21.6284                      |  | 1077                            | 25.069                       |
| 1076                            | 21.6164                      |  | 1076                            | 25.048                       |
| 1075                            | 21.5873                      |  | 1075                            | 25.0447                      |
| 1074                            | 21.5711                      |  | 1074                            | 25.0462                      |

## FIG. 56

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1073                            | 21.5786                      |  | 1073                            | 25.0449                      |
| 1072                            | 21.5785                      |  | 1072                            | 25.0508                      |
| 1071                            | 21.6013                      |  | 1071                            | 25.0541                      |
| 1070                            | 21.5906                      |  | 1070                            | 25.0465                      |
| 1069                            | 21.5785                      |  | 1069                            | 25.0455                      |
| 1068                            | 21.5927                      |  | 1068                            | 25.0463                      |
| 1067                            | 21.5798                      |  | 1067                            | 25.0278                      |
| 1066                            | 21.5966                      |  | 1066                            | 25.0289                      |
| 1065                            | 21.6195                      |  | 1065                            | 25.0419                      |
| 1064                            | 21.608                       |  | 1064                            | 25.0387                      |
| 1063                            | 21.6074                      |  | 1063                            | 25.0553                      |
| 1062                            | 21.6099                      |  | 1062                            | 25.068                       |
| 1061                            | 21.5858                      |  | 1061                            | 25.0516                      |
| 1060                            | 21.6045                      |  | 1060                            | 25.0646                      |
| 1059                            | 21.6155                      |  | 1059                            | 25.0569                      |
| 1058                            | 21.6223                      |  | 1058                            | 25.0611                      |
| 1057                            | 21.6271                      |  | 1057                            | 25.0467                      |
| 1056                            | 21.6316                      |  | 1056                            | 25.0507                      |
| 1055                            | 21.6328                      |  | 1055                            | 25.074                       |
| 1054                            | 21.6288                      |  | 1054                            | 25.0587                      |
| 1053                            | 21.6382                      |  | 1053                            | 25.0723                      |
| 1052                            | 21.6205                      |  | 1052                            | 25.0739                      |
| 1051                            | 21.6108                      |  | 1051                            | 25.0598                      |
| 1050                            | 21.612                       |  | 1050                            | 25.0618                      |
| 1049                            | 21.614                       |  | 1049                            | 25.0577                      |
| 1048                            | 21.6167                      |  | 1048                            | 25.0474                      |
| 1047                            | 21.6096                      |  | 1047                            | 25.0396                      |
| 1046                            | 21.592                       |  | 1046                            | 25.0458                      |

## FIG. 57

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1045                            | 21.5755                      |  | 1045                            | 25.0403                      |
| 1044                            | 21.5637                      |  | 1044                            | 25.0447                      |
| 1043                            | 21.577                       |  | 1043                            | 25.0413                      |
| 1042                            | 21.587                       |  | 1042                            | 25.0207                      |
| 1041                            | 21.583                       |  | 1041                            | 25.0082                      |
| 1040                            | 21.6093                      |  | 1040                            | 25.0012                      |
| 1039                            | 21.5941                      |  | 1039                            | 25.003                       |
| 1038                            | 21.5864                      |  | 1038                            | 25.0045                      |
| 1037                            | 21.5871                      |  | 1037                            | 25.0281                      |
| 1036                            | 21.5713                      |  | 1036                            | 25.0253                      |
| 1035                            | 21.5794                      |  | 1035                            | 25.008                       |
| 1034                            | 21.5653                      |  | 1034                            | 25.0093                      |
| 1033                            | 21.5632                      |  | 1033                            | 24.98                        |
| 1032                            | 21.562                       |  | 1032                            | 24.9869                      |
| 1031                            | 21.5638                      |  | 1031                            | 24.9937                      |
| 1030                            | 21.5743                      |  | 1030                            | 25.0174                      |
| 1029                            | 21.5892                      |  | 1029                            | 25.0482                      |
| 1028                            | 21.5731                      |  | 1028                            | 25.0299                      |
| 1027                            | 21.5663                      |  | 1027                            | 25.031                       |
| 1026                            | 21.5617                      |  | 1026                            | 25.0193                      |
| 1025                            | 21.5404                      |  | 1025                            | 24.9949                      |
| 1024                            | 21.5507                      |  | 1024                            | 24.9994                      |
| 1023                            | 21.5583                      |  | 1023                            | 25.002                       |
| 1022                            | 21.5666                      |  | 1022                            | 24.9992                      |
| 1021                            | 21.5565                      |  | 1021                            | 25.001                       |
| 1020                            | 21.5428                      |  | 1020                            | 25.0052                      |
| 1019                            | 21.5284                      |  | 1019                            | 24.9936                      |
| 1018                            | 21.5311                      |  | 1018                            | 24.9808                      |

## FIG. 58

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 1017                            | 21.5614                      |  | 1017                            | 24.9953                      |
| 1016                            | 21.5644                      |  | 1016                            | 24.9885                      |
| 1015                            | 21.5671                      |  | 1015                            | 25.0069                      |
| 1014                            | 21.5613                      |  | 1014                            | 25.0085                      |
| 1013                            | 21.5487                      |  | 1013                            | 24.999                       |
| 1012                            | 21.5536                      |  | 1012                            | 24.9885                      |
| 1011                            | 21.5683                      |  | 1011                            | 24.9909                      |
| 1010                            | 21.5822                      |  | 1010                            | 24.9939                      |
| 1009                            | 21.585                       |  | 1009                            | 24.9986                      |
| 1008                            | 21.5765                      |  | 1008                            | 25.0079                      |
| 1007                            | 21.55                        |  | 1007                            | 24.9923                      |
| 1006                            | 21.5281                      |  | 1006                            | 24.9875                      |
| 1005                            | 21.5077                      |  | 1005                            | 24.97                        |
| 1004                            | 21.5237                      |  | 1004                            | 24.9684                      |
| 1003                            | 21.5181                      |  | 1003                            | 24.9555                      |
| 1002                            | 21.5243                      |  | 1002                            | 24.9622                      |
| 1001                            | 21.5353                      |  | 1001                            | 24.9665                      |
| 1000                            | 21.5266                      |  | 1000                            | 24.9653                      |
| 999                             | 21.5488                      |  | 999                             | 24.9612                      |
| 998                             | 21.5529                      |  | 998                             | 24.9482                      |
| 997                             | 21.5474                      |  | 997                             | 24.9581                      |
| 996                             | 21.5294                      |  | 996                             | 24.9551                      |
| 995                             | 21.5276                      |  | 995                             | 24.9707                      |
| 994                             | 21.5356                      |  | 994                             | 24.9688                      |
| 993                             | 21.5236                      |  | 993                             | 24.9509                      |
| 992                             | 21.5344                      |  | 992                             | 24.9452                      |
| 991                             | 21.5303                      |  | 991                             | 24.9334                      |
| 990                             | 21.5202                      |  | 990                             | 24.9572                      |

## FIG. 59

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 989                             | 21.5344                      |  | 989                             | 24.9521                      |
| 988                             | 21.5388                      |  | 988                             | 24.9493                      |
| 987                             | 21.5394                      |  | 987                             | 24.9508                      |
| 986                             | 21.5275                      |  | 986                             | 24.924                       |
| 985                             | 21.5068                      |  | 985                             | 24.9368                      |
| 984                             | 21.498                       |  | 984                             | 24.9274                      |
| 983                             | 21.5027                      |  | 983                             | 24.9388                      |
| 982                             | 21.496                       |  | 982                             | 24.9271                      |
| 981                             | 21.5178                      |  | 981                             | 24.9264                      |
| 980                             | 21.5413                      |  | 980                             | 24.9476                      |
| 979                             | 21.5301                      |  | 979                             | 24.9402                      |
| 978                             | 21.551                       |  | 978                             | 24.9656                      |
| 977                             | 21.5514                      |  | 977                             | 24.9679                      |
| 976                             | 21.5343                      |  | 976                             | 24.9453                      |
| 975                             | 21.526                       |  | 975                             | 24.9419                      |
| 974                             | 21.5229                      |  | 974                             | 24.94                        |
| 973                             | 21.5044                      |  | 973                             | 24.9055                      |
| 972                             | 21.4949                      |  | 972                             | 24.9017                      |
| 971                             | 21.4831                      |  | 971                             | 24.8828                      |
| 970                             | 21.4521                      |  | 970                             | 24.8667                      |
| 969                             | 21.4412                      |  | 969                             | 24.8735                      |
| 968                             | 21.4528                      |  | 968                             | 24.8843                      |
| 967                             | 21.4446                      |  | 967                             | 24.8881                      |
| 966                             | 21.4583                      |  | 966                             | 24.8778                      |
| 965                             | 21.4588                      |  | 965                             | 24.8861                      |
| 964                             | 21.4525                      |  | 964                             | 24.8666                      |
| 963                             | 21.4741                      |  | 963                             | 24.8761                      |
| 962                             | 21.4767                      |  | 962                             | 24.8812                      |

## FIG. 60

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 961                             | 21.4813                      |  | 961                             | 24.873                       |
| 960                             | 21.4726                      |  | 960                             | 24.8778                      |
| 959                             | 21.4717                      |  | 959                             | 24.8864                      |
| 958                             | 21.4574                      |  | 958                             | 24.8771                      |
| 957                             | 21.4724                      |  | 957                             | 24.8739                      |
| 956                             | 21.467                       |  | 956                             | 24.8623                      |
| 955                             | 21.4574                      |  | 955                             | 24.8417                      |
| 954                             | 21.4489                      |  | 954                             | 24.8371                      |
| 953                             | 21.4455                      |  | 953                             | 24.8591                      |
| 952                             | 21.4322                      |  | 952                             | 24.8868                      |
| 951                             | 21.4492                      |  | 951                             | 24.8991                      |
| 950                             | 21.474                       |  | 950                             | 24.9138                      |
| 949                             | 21.504                       |  | 949                             | 24.9188                      |
| 948                             | 21.5404                      |  | 948                             | 24.9372                      |
| 947                             | 21.5529                      |  | 947                             | 24.9465                      |
| 946                             | 21.5737                      |  | 946                             | 24.9462                      |
| 945                             | 21.5488                      |  | 945                             | 24.9399                      |
| 944                             | 21.5454                      |  | 944                             | 24.9225                      |
| 943                             | 21.4998                      |  | 943                             | 24.9237                      |
| 942                             | 21.4772                      |  | 942                             | 24.9149                      |
| 941                             | 21.4823                      |  | 941                             | 24.9358                      |
| 940                             | 21.4798                      |  | 940                             | 24.9257                      |
| 939                             | 21.4885                      |  | 939                             | 24.9136                      |
| 938                             | 21.5172                      |  | 938                             | 24.9528                      |
| 937                             | 21.5143                      |  | 937                             | 24.9391                      |
| 936                             | 21.5011                      |  | 936                             | 24.9352                      |
| 935                             | 21.5097                      |  | 935                             | 24.9708                      |
| 934                             | 21.4854                      |  | 934                             | 24.942                       |

## FIG. 61

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 933                             | 21.468                       |  | 933                             | 24.923                       |
| 932                             | 21.4751                      |  | 932                             | 24.9304                      |
| 931                             | 21.5074                      |  | 931                             | 24.9093                      |
| 930                             | 21.4938                      |  | 930                             | 24.9038                      |
| 929                             | 21.4917                      |  | 929                             | 24.9161                      |
| 928                             | 21.4737                      |  | 928                             | 24.9054                      |
| 927                             | 21.4472                      |  | 927                             | 24.8893                      |
| 926                             | 21.459                       |  | 926                             | 24.8867                      |
| 925                             | 21.4385                      |  | 925                             | 24.842                       |
| 924                             | 21.4562                      |  | 924                             | 24.8499                      |
| 923                             | 21.4454                      |  | 923                             | 24.8403                      |
| 922                             | 21.4264                      |  | 922                             | 24.8356                      |
| 921                             | 21.4411                      |  | 921                             | 24.8763                      |
| 920                             | 21.4423                      |  | 920                             | 24.8923                      |
| 919                             | 21.4696                      |  | 919                             | 24.8791                      |
| 918                             | 21.4901                      |  | 918                             | 24.9016                      |
| 917                             | 21.5114                      |  | 917                             | 24.893                       |
| 916                             | 21.5094                      |  | 916                             | 24.8747                      |
| 915                             | 21.4669                      |  | 915                             | 24.8915                      |
| 914                             | 21.4267                      |  | 914                             | 24.8667                      |
| 913                             | 21.4332                      |  | 913                             | 24.8551                      |
| 912                             | 21.4222                      |  | 912                             | 24.831                       |
| 911                             | 21.4316                      |  | 911                             | 24.8023                      |
| 910                             | 21.4713                      |  | 910                             | 24.8174                      |
| 909                             | 21.4367                      |  | 909                             | 24.8461                      |
| 908                             | 21.4457                      |  | 908                             | 24.8569                      |
| 907                             | 21.4608                      |  | 907                             | 24.8578                      |
| 906                             | 21.4242                      |  | 906                             | 24.8665                      |

## FIG. 62

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 905                             | 21.4397                      |  | 905                             | 24.8166                      |
| 904                             | 21.4452                      |  | 904                             | 24.8143                      |
| 903                             | 21.4255                      |  | 903                             | 24.8228                      |
| 902                             | 21.4558                      |  | 902                             | 24.7668                      |
| 901                             | 21.4342                      |  | 901                             | 24.7997                      |
| 900                             | 21.4353                      |  | 900                             | 24.8035                      |
| 899                             | 21.4446                      |  | 899                             | 24.8013                      |
| 898                             | 21.4657                      |  | 898                             | 24.8037                      |
| 897                             | 21.4372                      |  | 897                             | 24.7695                      |
| 896                             | 21.3983                      |  | 896                             | 24.7455                      |
| 895                             | 21.4273                      |  | 895                             | 24.7804                      |
| 894                             | 21.3995                      |  | 894                             | 24.796                       |
| 893                             | 21.4492                      |  | 893                             | 24.8016                      |
| 892                             | 21.4703                      |  | 892                             | 24.8182                      |
| 891                             | 21.4496                      |  | 891                             | 24.792                       |
| 890                             | 21.4145                      |  | 890                             | 24.7998                      |
| 889                             | 21.3915                      |  | 889                             | 24.8307                      |
| 888                             | 21.401                       |  | 888                             | 24.8401                      |
| 887                             | 21.3627                      |  | 887                             | 24.8382                      |
| 886                             | 21.3607                      |  | 886                             | 24.8113                      |
| 885                             | 21.3801                      |  | 885                             | 24.7936                      |
| 884                             | 21.3341                      |  | 884                             | 24.7487                      |
| 883                             | 21.3689                      |  | 883                             | 24.7234                      |
| 882                             | 21.4067                      |  | 882                             | 24.7433                      |
| 881                             | 21.3838                      |  | 881                             | 24.7465                      |
| 880                             | 21.4505                      |  | 880                             | 24.7738                      |
| 879                             | 21.4538                      |  | 879                             | 24.798                       |
| 878                             | 21.443                       |  | 878                             | 24.8269                      |

## FIG. 63

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 877                             | 21.4947                      |  | 877                             | 24.7763                      |
| 876                             | 21.3778                      |  | 876                             | 24.7541                      |
| 875                             | 21.3631                      |  | 875                             | 24.7277                      |
| 874                             | 21.376                       |  | 874                             | 24.7182                      |
| 873                             | 21.3965                      |  | 873                             | 24.8024                      |
| 872                             | 21.5281                      |  | 872                             | 24.8899                      |
| 871                             | 21.5382                      |  | 871                             | 24.9218                      |
| 870                             | 21.5277                      |  | 870                             | 24.8819                      |
| 869                             | 21.4457                      |  | 869                             | 24.8705                      |
| 868                             | 21.4251                      |  | 868                             | 24.8191                      |
| 867                             | 21.4229                      |  | 867                             | 24.8147                      |
| 866                             | 21.3965                      |  | 866                             | 24.842                       |
| 865                             | 21.4025                      |  | 865                             | 24.8191                      |
| 864                             | 21.3544                      |  | 864                             | 24.8468                      |
| 863                             | 21.3196                      |  | 863                             | 24.8904                      |
| 862                             | 21.3217                      |  | 862                             | 24.8734                      |
| 861                             | 21.3167                      |  | 861                             | 24.8452                      |
| 860                             | 21.7633                      |  | 860                             | 24.836                       |
| 859                             | 21.6386                      |  | 859                             | 25.0196                      |
| 858                             | 21.8014                      |  | 858                             | 25.0867                      |
| 857                             | 21.758                       |  | 857                             | 25.0826                      |
| 856                             | 21.8537                      |  | 856                             | 25.1822                      |
| 855                             | 21.958                       |  | 855                             | 25.0755                      |
| 854                             | 21.7795                      |  | 854                             | 24.98                        |
| 853                             | 21.8385                      |  | 853                             | 24.9235                      |
| 852                             | 21.8652                      |  | 852                             | 24.8336                      |
| 851                             | 21.679                       |  | 851                             | 24.745                       |
| 850                             | 21.6637                      |  | 850                             | 24.5902                      |

## FIG. 64

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 849                             | 21.693                       |  | 849                             | 24.7719                      |
| 848                             | 21.6952                      |  | 848                             | 24.8626                      |
| 847                             | 21.7963                      |  | 847                             | 24.9778                      |
| 846                             | 21.8801                      |  | 846                             | 25.1357                      |
| 845                             | 21.8646                      |  | 845                             | 25.0127                      |
| 844                             | 21.7934                      |  | 844                             | 25.0418                      |
| 843                             | 21.6918                      |  | 843                             | 24.9604                      |
| 842                             | 21.7108                      |  | 842                             | 24.9613                      |
| 841                             | 21.6744                      |  | 841                             | 25.0892                      |
| 840                             | 21.6936                      |  | 840                             | 25.0393                      |
| 839                             | 21.7358                      |  | 839                             | 25.0136                      |
| 838                             | 21.6368                      |  | 838                             | 24.978                       |
| 837                             | 21.6987                      |  | 837                             | 24.9738                      |
| 836                             | 21.7044                      |  | 836                             | 24.9589                      |
| 835                             | 21.6588                      |  | 835                             | 25.0132                      |
| 834                             | 21.6984                      |  | 834                             | 25.0294                      |
| 833                             | 21.6341                      |  | 833                             | 24.9768                      |
| 832                             | 21.6308                      |  | 832                             | 24.993                       |
| 831                             | 21.6584                      |  | 831                             | 24.9696                      |
| 830                             | 21.5967                      |  | 830                             | 24.9567                      |
| 829                             | 21.5364                      |  | 829                             | 24.9208                      |
| 828                             | 21.5311                      |  | 828                             | 24.9074                      |
| 827                             | 21.4683                      |  | 827                             | 24.9342                      |
| 826                             | 21.5379                      |  | 826                             | 24.9536                      |
| 825                             | 21.5708                      |  | 825                             | 25.0148                      |
| 824                             | 21.5142                      |  | 824                             | 25.0315                      |
| 823                             | 21.4925                      |  | 823                             | 25.0147                      |
| 822                             | 21.4677                      |  | 822                             | 25.0456                      |

## FIG. 65

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 821                             | 21.4652                      |  | 821                             | 25.0278                      |
| 820                             | 21.5186                      |  | 820                             | 25.0013                      |
| 819                             | 21.537                       |  | 819                             | 24.9879                      |
| 818                             | 21.5177                      |  | 818                             | 24.9388                      |
| 817                             | 21.5577                      |  | 817                             | 24.9254                      |
| 816                             | 21.5471                      |  | 816                             | 24.9341                      |
| 815                             | 21.5615                      |  | 815                             | 24.9565                      |
| 814                             | 21.5683                      |  | 814                             | 24.8965                      |
| 813                             | 21.5633                      |  | 813                             | 24.8981                      |
| 812                             | 21.5354                      |  | 812                             | 24.8769                      |
| 811                             | 21.5425                      |  | 811                             | 24.8373                      |
| 810                             | 21.5548                      |  | 810                             | 24.87                        |
| 809                             | 21.5101                      |  | 809                             | 24.8381                      |
| 808                             | 21.5605                      |  | 808                             | 24.8624                      |
| 807                             | 21.5736                      |  | 807                             | 24.855                       |
| 806                             | 21.5517                      |  | 806                             | 24.8515                      |
| 805                             | 21.5789                      |  | 805                             | 24.8551                      |
| 804                             | 21.5532                      |  | 804                             | 24.8153                      |
| 803                             | 21.5637                      |  | 803                             | 24.8474                      |
| 802                             | 21.5738                      |  | 802                             | 24.864                       |
| 801                             | 21.5593                      |  | 801                             | 24.8754                      |
| 800                             | 21.5647                      |  | 800                             | 24.8998                      |
| 799                             | 21.5183                      |  | 799                             | 24.8947                      |
| 798                             | 21.5136                      |  | 798                             | 24.9065                      |
| 797                             | 21.5369                      |  | 797                             | 24.924                       |
| 796                             | 21.5233                      |  | 796                             | 24.9067                      |
| 795                             | 21.5769                      |  | 795                             | 24.9054                      |
| 794                             | 21.5968                      |  | 794                             | 24.9088                      |

## FIG. 66

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 793                             | 21.581                       |  | 793                             | 24.8777                      |
| 792                             | 21.6154                      |  | 792                             | 24.8939                      |
| 791                             | 21.5646                      |  | 791                             | 24.8754                      |
| 790                             | 21.5637                      |  | 790                             | 24.833                       |
| 789                             | 21.5652                      |  | 789                             | 24.8563                      |
| 788                             | 21.5381                      |  | 788                             | 24.8348                      |
| 787                             | 21.549                       |  | 787                             | 24.8208                      |
| 786                             | 21.555                       |  | 786                             | 24.8479                      |
| 785                             | 21.5417                      |  | 785                             | 24.832                       |
| 784                             | 21.5333                      |  | 784                             | 24.8231                      |
| 783                             | 21.536                       |  | 783                             | 24.8508                      |
| 782                             | 21.4895                      |  | 782                             | 24.8179                      |
| 781                             | 21.4752                      |  | 781                             | 24.7747                      |
| 780                             | 21.5254                      |  | 780                             | 24.7975                      |
| 779                             | 21.4953                      |  | 779                             | 24.7902                      |
| 778                             | 21.4713                      |  | 778                             | 24.8003                      |
| 777                             | 21.5088                      |  | 777                             | 24.8353                      |
| 776                             | 21.4574                      |  | 776                             | 24.8491                      |
| 775                             | 21.4845                      |  | 775                             | 24.8123                      |
| 774                             | 21.4867                      |  | 774                             | 24.813                       |
| 773                             | 21.441                       |  | 773                             | 24.8146                      |
| 772                             | 21.4717                      |  | 772                             | 24.8258                      |
| 771                             | 21.4513                      |  | 771                             | 24.8745                      |
| 770                             | 21.4758                      |  | 770                             | 24.874                       |
| 769                             | 21.5148                      |  | 769                             | 24.861                       |
| 768                             | 21.499                       |  | 768                             | 24.8115                      |
| 767                             | 21.5234                      |  | 767                             | 24.8281                      |
| 766                             | 21.5225                      |  | 766                             | 24.8725                      |

## FIG. 67

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 765                             | 21.4771                      |  | 765                             | 24.8714                      |
| 764                             | 21.4768                      |  | 764                             | 24.8934                      |
| 763                             | 21.4518                      |  | 763                             | 24.8607                      |
| 762                             | 21.4729                      |  | 762                             | 24.8106                      |
| 761                             | 21.4885                      |  | 761                             | 24.7934                      |
| 760                             | 21.4741                      |  | 760                             | 24.779                       |
| 759                             | 21.4903                      |  | 759                             | 24.7575                      |
| 758                             | 21.461                       |  | 758                             | 24.75                        |
| 757                             | 21.4456                      |  | 757                             | 24.7377                      |
| 756                             | 21.4785                      |  | 756                             | 24.7625                      |
| 755                             | 21.4713                      |  | 755                             | 24.7825                      |
| 754                             | 21.4805                      |  | 754                             | 24.8228                      |
| 753                             | 21.4803                      |  | 753                             | 24.8317                      |
| 752                             | 21.4543                      |  | 752                             | 24.8506                      |
| 751                             | 21.4366                      |  | 751                             | 24.8358                      |
| 750                             | 21.4125                      |  | 750                             | 24.79                        |
| 749                             | 21.4172                      |  | 749                             | 24.7813                      |
| 748                             | 21.421                       |  | 748                             | 24.7192                      |
| 747                             | 21.4345                      |  | 747                             | 24.7382                      |
| 746                             | 21.4504                      |  | 746                             | 24.7601                      |
| 745                             | 21.4502                      |  | 745                             | 24.7896                      |
| 744                             | 21.4296                      |  | 744                             | 24.7942                      |
| 743                             | 21.4249                      |  | 743                             | 24.7834                      |
| 742                             | 21.4203                      |  | 742                             | 24.7693                      |
| 741                             | 21.442                       |  | 741                             | 24.7867                      |
| 740                             | 21.45                        |  | 740                             | 24.8082                      |
| 739                             | 21.4525                      |  | 739                             | 24.8044                      |
| 738                             | 21.4575                      |  | 738                             | 24.806                       |

## FIG. 68

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 737                             | 21.4489                      |  | 737                             | 24.8025                      |
| 736                             | 21.4297                      |  | 736                             | 24.8034                      |
| 735                             | 21.3993                      |  | 735                             | 24.8166                      |
| 734                             | 21.3692                      |  | 734                             | 24.8202                      |
| 733                             | 21.3714                      |  | 733                             | 24.8015                      |
| 732                             | 21.3657                      |  | 732                             | 24.7858                      |
| 731                             | 21.3837                      |  | 731                             | 24.7725                      |
| 730                             | 21.394                       |  | 730                             | 24.7717                      |
| 729                             | 21.3745                      |  | 729                             | 24.7797                      |
| 728                             | 21.3872                      |  | 728                             | 24.7792                      |
| 727                             | 21.3692                      |  | 727                             | 24.7841                      |
| 726                             | 21.3438                      |  | 726                             | 24.7838                      |
| 725                             | 21.3611                      |  | 725                             | 24.8149                      |
| 724                             | 21.3414                      |  | 724                             | 24.8274                      |
| 723                             | 21.3388                      |  | 723                             | 24.8118                      |
| 722                             | 21.3465                      |  | 722                             | 24.81                        |
| 721                             | 21.3434                      |  | 721                             | 24.7825                      |
| 720                             | 21.3376                      |  | 720                             | 24.7784                      |
| 719                             | 21.3339                      |  | 719                             | 24.789                       |
| 718                             | 21.3231                      |  | 718                             | 24.7648                      |
| 717                             | 21.2891                      |  | 717                             | 24.7477                      |
| 716                             | 21.279                       |  | 716                             | 24.7344                      |
| 715                             | 21.2775                      |  | 715                             | 24.7253                      |
| 714                             | 21.2548                      |  | 714                             | 24.7181                      |
| 713                             | 21.2605                      |  | 713                             | 24.7112                      |
| 712                             | 21.2529                      |  | 712                             | 24.7066                      |
| 711                             | 21.2536                      |  | 711                             | 24.7067                      |
| 710                             | 21.2481                      |  | 710                             | 24.718                       |

## FIG. 69

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 709                             | 21.2198                      |  | 709                             | 24.72                        |
| 708                             | 21.2194                      |  | 708                             | 24.7278                      |
| 707                             | 21.1865                      |  | 707                             | 24.7243                      |
| 706                             | 21.1876                      |  | 706                             | 24.7357                      |
| 705                             | 21.2013                      |  | 705                             | 24.7492                      |
| 704                             | 21.1818                      |  | 704                             | 24.7503                      |
| 703                             | 21.1792                      |  | 703                             | 24.7627                      |
| 702                             | 21.1642                      |  | 702                             | 24.7671                      |
| 701                             | 21.1494                      |  | 701                             | 24.7694                      |
| 700                             | 21.1342                      |  | 700                             | 24.7717                      |
| 699                             | 21.1225                      |  | 699                             | 24.7643                      |
| 698                             | 21.1086                      |  | 698                             | 24.7623                      |
| 697                             | 21.0837                      |  | 697                             | 24.7646                      |
| 696                             | 21.0717                      |  | 696                             | 24.7547                      |
| 695                             | 21.0457                      |  | 695                             | 24.7339                      |
| 694                             | 21.016                       |  | 694                             | 24.7139                      |
| 693                             | 20.9966                      |  | 693                             | 24.6915                      |
| 692                             | 20.9752                      |  | 692                             | 24.6987                      |
| 691                             | 20.94                        |  | 691                             | 24.6871                      |
| 690                             | 20.915                       |  | 690                             | 24.6699                      |
| 689                             | 20.8837                      |  | 689                             | 24.661                       |
| 688                             | 20.8437                      |  | 688                             | 24.6243                      |
| 687                             | 20.8222                      |  | 687                             | 24.6276                      |
| 686                             | 20.793                       |  | 686                             | 24.6042                      |
| 685                             | 20.7591                      |  | 685                             | 24.5667                      |
| 684                             | 20.7286                      |  | 684                             | 24.5564                      |
| 683                             | 20.6989                      |  | 683                             | 24.5383                      |
| 682                             | 20.6696                      |  | 682                             | 24.5572                      |

## FIG. 70

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 681                             | 20.6588                      |  | 681                             | 24.5852                      |
| 680                             | 20.6341                      |  | 680                             | 24.5838                      |
| 679                             | 20.6234                      |  | 679                             | 24.5739                      |
| 678                             | 20.6385                      |  | 678                             | 24.5831                      |
| 677                             | 20.6513                      |  | 677                             | 24.605                       |
| 676                             | 20.6697                      |  | 676                             | 24.6485                      |
| 675                             | 20.6734                      |  | 675                             | 24.6815                      |
| 674                             | 20.6486                      |  | 674                             | 24.6948                      |
| 673                             | 20.6107                      |  | 673                             | 24.6888                      |
| 672                             | 20.5911                      |  | 672                             | 24.6787                      |
| 671                             | 20.576                       |  | 671                             | 24.6793                      |
| 670                             | 20.5519                      |  | 670                             | 24.6606                      |
| 669                             | 20.525                       |  | 669                             | 24.6348                      |
| 668                             | 20.4925                      |  | 668                             | 24.6155                      |
| 667                             | 20.4808                      |  | 667                             | 24.6158                      |
| 666                             | 20.4831                      |  | 666                             | 24.6185                      |
| 665                             | 20.4851                      |  | 665                             | 24.6491                      |
| 664                             | 20.4819                      |  | 664                             | 24.6626                      |
| 663                             | 20.4553                      |  | 663                             | 24.6651                      |
| 662                             | 20.4474                      |  | 662                             | 24.6552                      |
| 661                             | 20.4445                      |  | 661                             | 24.6449                      |
| 660                             | 20.437                       |  | 660                             | 24.6419                      |
| 659                             | 20.4152                      |  | 659                             | 24.6259                      |
| 658                             | 20.3931                      |  | 658                             | 24.627                       |
| 657                             | 20.3656                      |  | 657                             | 24.6127                      |
| 656                             | 20.3722                      |  | 656                             | 24.6321                      |
| 655                             | 20.384                       |  | 655                             | 24.6386                      |
| 654                             | 20.3734                      |  | 654                             | 24.6475                      |

## FIG. 71

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 653                             | 20.3862                      |  | 653                             | 24.6725                      |
| 652                             | 20.3457                      |  | 652                             | 24.6476                      |
| 651                             | 20.3306                      |  | 651                             | 24.6404                      |
| 650                             | 20.3179                      |  | 650                             | 24.648                       |
| 649                             | 20.2836                      |  | 649                             | 24.627                       |
| 648                             | 20.2686                      |  | 648                             | 24.5876                      |
| 647                             | 20.2599                      |  | 647                             | 24.5942                      |
| 646                             | 20.2608                      |  | 646                             | 24.5802                      |
| 645                             | 20.273                       |  | 645                             | 24.5976                      |
| 644                             | 20.2727                      |  | 644                             | 24.6139                      |
| 643                             | 20.2651                      |  | 643                             | 24.6113                      |
| 642                             | 20.2598                      |  | 642                             | 24.6055                      |
| 641                             | 20.2476                      |  | 641                             | 24.5658                      |
| 640                             | 20.247                       |  | 640                             | 24.5688                      |
| 639                             | 20.2408                      |  | 639                             | 24.5663                      |
| 638                             | 20.2372                      |  | 638                             | 24.5853                      |
| 637                             | 20.2352                      |  | 637                             | 24.6043                      |
| 636                             | 20.2367                      |  | 636                             | 24.6214                      |
| 635                             | 20.2415                      |  | 635                             | 24.6348                      |
| 634                             | 20.24                        |  | 634                             | 24.6159                      |
| 633                             | 20.2222                      |  | 633                             | 24.6188                      |
| 632                             | 20.2241                      |  | 632                             | 24.6133                      |
| 631                             | 20.2161                      |  | 631                             | 24.607                       |
| 630                             | 20.198                       |  | 630                             | 24.6052                      |
| 629                             | 20.2047                      |  | 629                             | 24.5949                      |
| 628                             | 20.1965                      |  | 628                             | 24.5915                      |
| 627                             | 20.1946                      |  | 627                             | 24.5817                      |
| 626                             | 20.197                       |  | 626                             | 24.5806                      |

## FIG. 72

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 625                             | 20.195                       |  | 625                             | 24.5844                      |
| 624                             | 20.2006                      |  | 624                             | 24.5922                      |
| 623                             | 20.2031                      |  | 623                             | 24.6114                      |
| 622                             | 20.2099                      |  | 622                             | 24.6177                      |
| 621                             | 20.2177                      |  | 621                             | 24.6193                      |
| 620                             | 20.2124                      |  | 620                             | 24.6201                      |
| 619                             | 20.2015                      |  | 619                             | 24.592                       |
| 618                             | 20.1947                      |  | 618                             | 24.5912                      |
| 617                             | 20.1874                      |  | 617                             | 24.6052                      |
| 616                             | 20.1673                      |  | 616                             | 24.5988                      |
| 615                             | 20.1611                      |  | 615                             | 24.6007                      |
| 614                             | 20.1501                      |  | 614                             | 24.5943                      |
| 613                             | 20.1369                      |  | 613                             | 24.584                       |
| 612                             | 20.156                       |  | 612                             | 24.5851                      |
| 611                             | 20.1558                      |  | 611                             | 24.5903                      |
| 610                             | 20.165                       |  | 610                             | 24.6053                      |
| 609                             | 20.1626                      |  | 609                             | 24.6013                      |
| 608                             | 20.1606                      |  | 608                             | 24.5913                      |
| 607                             | 20.1631                      |  | 607                             | 24.5784                      |
| 606                             | 20.1568                      |  | 606                             | 24.5528                      |
| 605                             | 20.1639                      |  | 605                             | 24.5499                      |
| 604                             | 20.1517                      |  | 604                             | 24.5267                      |
| 603                             | 20.1502                      |  | 603                             | 24.5289                      |
| 602                             | 20.1422                      |  | 602                             | 24.5371                      |
| 601                             | 20.1232                      |  | 601                             | 24.5256                      |
| 600                             | 20.1595                      |  | 600                             | 24.569                       |
| 599                             | 20.1618                      |  | 599                             | 24.5583                      |
| 598                             | 20.1483                      |  | 598                             | 24.5577                      |

## FIG. 73

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 597                             | 20.1493                      |  | 597                             | 24.5644                      |
| 596                             | 20.1652                      |  | 596                             | 24.561                       |
| 595                             | 20.161                       |  | 595                             | 24.5611                      |
| 594                             | 20.1779                      |  | 594                             | 24.5646                      |
| 593                             | 20.1828                      |  | 593                             | 24.5528                      |
| 592                             | 20.1788                      |  | 592                             | 24.565                       |
| 591                             | 20.1904                      |  | 591                             | 24.5714                      |
| 590                             | 20.1929                      |  | 590                             | 24.5669                      |
| 589                             | 20.1808                      |  | 589                             | 24.5679                      |
| 588                             | 20.1703                      |  | 588                             | 24.5621                      |
| 587                             | 20.1571                      |  | 587                             | 24.5416                      |
| 586                             | 20.1462                      |  | 586                             | 24.5336                      |
| 585                             | 20.1412                      |  | 585                             | 24.5247                      |
| 584                             | 20.1461                      |  | 584                             | 24.5314                      |
| 583                             | 20.1488                      |  | 583                             | 24.5508                      |
| 582                             | 20.151                       |  | 582                             | 24.5573                      |
| 581                             | 20.1583                      |  | 581                             | 24.5483                      |
| 580                             | 20.1439                      |  | 580                             | 24.5378                      |
| 579                             | 20.1484                      |  | 579                             | 24.5434                      |
| 578                             | 20.1437                      |  | 578                             | 24.5464                      |
| 577                             | 20.1603                      |  | 577                             | 24.5603                      |
| 576                             | 20.1699                      |  | 576                             | 24.5567                      |
| 575                             | 20.1781                      |  | 575                             | 24.5468                      |
| 574                             | 20.2004                      |  | 574                             | 24.5497                      |
| 573                             | 20.199                       |  | 573                             | 24.5596                      |
| 572                             | 20.209                       |  | 572                             | 24.5562                      |
| 571                             | 20.1872                      |  | 571                             | 24.5555                      |
| 570                             | 20.1861                      |  | 570                             | 24.534                       |

## FIG. 74

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 569                             | 20.1814                      |  | 569                             | 24.5307                      |
| 568                             | 20.1729                      |  | 568                             | 24.5283                      |
| 567                             | 20.1869                      |  | 567                             | 24.5381                      |
| 566                             | 20.1836                      |  | 566                             | 24.5329                      |
| 565                             | 20.19                        |  | 565                             | 24.5209                      |
| 564                             | 20.1964                      |  | 564                             | 24.5234                      |
| 563                             | 20.2045                      |  | 563                             | 24.5007                      |
| 562                             | 20.2008                      |  | 562                             | 24.5156                      |
| 561                             | 20.1989                      |  | 561                             | 24.5298                      |
| 560                             | 20.2011                      |  | 560                             | 24.5352                      |
| 559                             | 20.2008                      |  | 559                             | 24.5447                      |
| 558                             | 20.2145                      |  | 558                             | 24.5615                      |
| 557                             | 20.2185                      |  | 557                             | 24.5341                      |
| 556                             | 20.2258                      |  | 556                             | 24.5199                      |
| 555                             | 20.2381                      |  | 555                             | 24.5131                      |
| 554                             | 20.2294                      |  | 554                             | 24.5068                      |
| 553                             | 20.2257                      |  | 553                             | 24.5228                      |
| 552                             | 20.2184                      |  | 552                             | 24.5256                      |
| 551                             | 20.2131                      |  | 551                             | 24.5403                      |
| 550                             | 20.2243                      |  | 550                             | 24.5391                      |
| 549                             | 20.2372                      |  | 549                             | 24.529                       |
| 548                             | 20.2569                      |  | 548                             | 24.5373                      |
| 547                             | 20.2539                      |  | 547                             | 24.5232                      |
| 546                             | 20.2515                      |  | 546                             | 24.513                       |
| 545                             | 20.247                       |  | 545                             | 24.5124                      |
| 544                             | 20.2386                      |  | 544                             | 24.5075                      |
| 543                             | 20.253                       |  | 543                             | 24.521                       |
| 542                             | 20.2539                      |  | 542                             | 24.5296                      |

## FIG. 75

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 541                             | 20.2593                      |  | 541                             | 24.526                       |
| 540                             | 20.2634                      |  | 540                             | 24.5242                      |
| 539                             | 20.2441                      |  | 539                             | 24.5217                      |
| 538                             | 20.2413                      |  | 538                             | 24.5108                      |
| 537                             | 20.2479                      |  | 537                             | 24.5207                      |
| 536                             | 20.2415                      |  | 536                             | 24.5317                      |
| 535                             | 20.2555                      |  | 535                             | 24.5094                      |
| 534                             | 20.2679                      |  | 534                             | 24.5083                      |
| 533                             | 20.2691                      |  | 533                             | 24.5055                      |
| 532                             | 20.2725                      |  | 532                             | 24.4893                      |
| 531                             | 20.276                       |  | 531                             | 24.4886                      |
| 530                             | 20.2669                      |  | 530                             | 24.4932                      |
| 529                             | 20.2592                      |  | 529                             | 24.4959                      |
| 528                             | 20.2623                      |  | 528                             | 24.4944                      |
| 527                             | 20.2488                      |  | 527                             | 24.5004                      |
| 526                             | 20.2517                      |  | 526                             | 24.4939                      |
| 525                             | 20.2495                      |  | 525                             | 24.4807                      |
| 524                             | 20.252                       |  | 524                             | 24.4883                      |
| 523                             | 20.2667                      |  | 523                             | 24.4963                      |
| 522                             | 20.2737                      |  | 522                             | 24.5038                      |
| 521                             | 20.2723                      |  | 521                             | 24.4977                      |
| 520                             | 20.285                       |  | 520                             | 24.5355                      |
| 519                             | 20.2935                      |  | 519                             | 24.5278                      |
| 518                             | 20.2934                      |  | 518                             | 24.5281                      |
| 517                             | 20.2879                      |  | 517                             | 24.5196                      |
| 516                             | 20.2852                      |  | 516                             | 24.5208                      |
| 515                             | 20.2749                      |  | 515                             | 24.5132                      |
| 514                             | 20.266                       |  | 514                             | 24.5149                      |

## FIG. 76

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 513                             | 20.2734                      |  | 513                             | 24.5115                      |
| 512                             | 20.2873                      |  | 512                             | 24.5035                      |
| 511                             | 20.2863                      |  | 511                             | 24.4997                      |
| 510                             | 20.2912                      |  | 510                             | 24.4902                      |
| 509                             | 20.2869                      |  | 509                             | 24.4864                      |
| 508                             | 20.2618                      |  | 508                             | 24.4829                      |
| 507                             | 20.2571                      |  | 507                             | 24.4649                      |
| 506                             | 20.2474                      |  | 506                             | 24.4652                      |
| 505                             | 20.2454                      |  | 505                             | 24.4714                      |
| 504                             | 20.2491                      |  | 504                             | 24.4827                      |
| 503                             | 20.2592                      |  | 503                             | 24.5087                      |
| 502                             | 20.2643                      |  | 502                             | 24.5059                      |
| 501                             | 20.2703                      |  | 501                             | 24.5262                      |
| 500                             | 20.2606                      |  | 500                             | 24.5208                      |
| 499                             | 20.2538                      |  | 499                             | 24.5275                      |
| 498                             | 20.2431                      |  | 498                             | 24.5274                      |
| 497                             | 20.2408                      |  | 497                             | 24.5016                      |
| 496                             | 20.2536                      |  | 496                             | 24.4963                      |
| 495                             | 20.2588                      |  | 495                             | 24.4814                      |
| 494                             | 20.27                        |  | 494                             | 24.4812                      |
| 493                             | 20.2655                      |  | 493                             | 24.4731                      |
| 492                             | 20.2701                      |  | 492                             | 24.4789                      |
| 491                             | 20.2705                      |  | 491                             | 24.4897                      |
| 490                             | 20.2674                      |  | 490                             | 24.4902                      |
| 489                             | 20.2783                      |  | 489                             | 24.5006                      |
| 488                             | 20.2706                      |  | 488                             | 24.5023                      |
| 487                             | 20.266                       |  | 487                             | 24.4879                      |
| 486                             | 20.2756                      |  | 486                             | 24.4963                      |

## FIG. 77

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 485                             | 20.2664                      |  | 485                             | 24.5003                      |
| 484                             | 20.2624                      |  | 484                             | 24.5048                      |
| 483                             | 20.2589                      |  | 483                             | 24.5107                      |
| 482                             | 20.2467                      |  | 482                             | 24.5108                      |
| 481                             | 20.2506                      |  | 481                             | 24.4998                      |
| 480                             | 20.2457                      |  | 480                             | 24.4864                      |
| 479                             | 20.2389                      |  | 479                             | 24.4755                      |
| 478                             | 20.2341                      |  | 478                             | 24.4569                      |
| 477                             | 20.233                       |  | 477                             | 24.4777                      |
| 476                             | 20.2455                      |  | 476                             | 24.4786                      |
| 475                             | 20.2711                      |  | 475                             | 24.4886                      |
| 474                             | 20.2748                      |  | 474                             | 24.4966                      |
| 473                             | 20.2699                      |  | 473                             | 24.4904                      |
| 472                             | 20.2562                      |  | 472                             | 24.4999                      |
| 471                             | 20.2455                      |  | 471                             | 24.5052                      |
| 470                             | 20.2454                      |  | 470                             | 24.5122                      |
| 469                             | 20.237                       |  | 469                             | 24.5083                      |
| 468                             | 20.2555                      |  | 468                             | 24.5078                      |
| 467                             | 20.2464                      |  | 467                             | 24.4957                      |
| 466                             | 20.2485                      |  | 466                             | 24.4988                      |
| 465                             | 20.2562                      |  | 465                             | 24.4947                      |
| 464                             | 20.2589                      |  | 464                             | 24.4802                      |
| 463                             | 20.2566                      |  | 463                             | 24.4842                      |
| 462                             | 20.2385                      |  | 462                             | 24.4546                      |
| 461                             | 20.2351                      |  | 461                             | 24.4543                      |
| 460                             | 20.2227                      |  | 460                             | 24.4401                      |
| 459                             | 20.224                       |  | 459                             | 24.448                       |
| 458                             | 20.2359                      |  | 458                             | 24.4615                      |

## FIG. 78

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 457                             | 20.2255                      |  | 457                             | 24.4513                      |
| 456                             | 20.2209                      |  | 456                             | 24.4576                      |
| 455                             | 20.2292                      |  | 455                             | 24.4581                      |
| 454                             | 20.2276                      |  | 454                             | 24.4508                      |
| 453                             | 20.2392                      |  | 453                             | 24.4583                      |
| 452                             | 20.2327                      |  | 452                             | 24.4604                      |
| 451                             | 20.2357                      |  | 451                             | 24.4427                      |
| 450                             | 20.2278                      |  | 450                             | 24.442                       |
| 449                             | 20.246                       |  | 449                             | 24.4422                      |
| 448                             | 20.2567                      |  | 448                             | 24.4527                      |
| 447                             | 20.24                        |  | 447                             | 24.4618                      |
| 446                             | 20.2605                      |  | 446                             | 24.4706                      |
| 445                             | 20.2502                      |  | 445                             | 24.4522                      |
| 444                             | 20.2491                      |  | 444                             | 24.4544                      |
| 443                             | 20.2706                      |  | 443                             | 24.462                       |
| 442                             | 20.2675                      |  | 442                             | 24.4668                      |
| 441                             | 20.2662                      |  | 441                             | 24.4815                      |
| 440                             | 20.2647                      |  | 440                             | 24.4846                      |
| 439                             | 20.255                       |  | 439                             | 24.4599                      |
| 438                             | 20.2474                      |  | 438                             | 24.4477                      |
| 437                             | 20.2518                      |  | 437                             | 24.4534                      |
| 436                             | 20.2708                      |  | 436                             | 24.4532                      |
| 435                             | 20.2768                      |  | 435                             | 24.4569                      |
| 434                             | 20.2944                      |  | 434                             | 24.4747                      |
| 433                             | 20.3071                      |  | 433                             | 24.4784                      |
| 432                             | 20.3026                      |  | 432                             | 24.4818                      |
| 431                             | 20.3069                      |  | 431                             | 24.5169                      |
| 430                             | 20.3146                      |  | 430                             | 24.528                       |

## FIG. 79

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 429                             | 20.3094                      |  | 429                             | 24.5347                      |
| 428                             | 20.3135                      |  | 428                             | 24.536                       |
| 427                             | 20.3431                      |  | 427                             | 24.5587                      |
| 426                             | 20.3436                      |  | 426                             | 24.5524                      |
| 425                             | 20.3452                      |  | 425                             | 24.5336                      |
| 424                             | 20.3365                      |  | 424                             | 24.5252                      |
| 423                             | 20.3023                      |  | 423                             | 24.4771                      |
| 422                             | 20.2883                      |  | 422                             | 24.4612                      |
| 421                             | 20.2542                      |  | 421                             | 24.4479                      |
| 420                             | 20.3519                      |  | 420                             | 24.5214                      |
| 419                             | 20.3317                      |  | 419                             | 24.5087                      |
| 418                             | 20.3461                      |  | 418                             | 24.4898                      |
| 417                             | 20.3088                      |  | 417                             | 24.5051                      |
| 416                             | 20.3093                      |  | 416                             | 24.4849                      |
| 415                             | 20.3189                      |  | 415                             | 24.4649                      |
| 414                             | 20.2861                      |  | 414                             | 24.418                       |
| 413                             | 20.3106                      |  | 413                             | 24.4366                      |
| 412                             | 20.3504                      |  | 412                             | 24.4542                      |
| 411                             | 20.3434                      |  | 411                             | 24.4923                      |
| 410                             | 20.3624                      |  | 410                             | 24.5297                      |
| 409                             | 20.3763                      |  | 409                             | 24.5202                      |
| 408                             | 20.3645                      |  | 408                             | 24.5415                      |
| 407                             | 20.4058                      |  | 407                             | 24.5158                      |
| 406                             | 20.4277                      |  | 406                             | 24.5275                      |
| 405                             | 20.4538                      |  | 405                             | 24.5364                      |
| 404                             | 20.4669                      |  | 404                             | 24.5238                      |
| 403                             | 20.4704                      |  | 403                             | 24.5375                      |
| 402                             | 20.4856                      |  | 402                             | 24.5262                      |

**FIG. 80**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 401                             | 20.4931                      |  | 401                             | 24.5059                      |
| 400                             | 20.4686                      |  | 400                             | 24.5008                      |
| 399                             | 20.4815                      |  | 399                             | 24.5177                      |
| 398                             | 20.4674                      |  | 398                             | 24.5491                      |
| 397                             | 20.4531                      |  | 397                             | 24.5543                      |
| 396                             | 20.4681                      |  | 396                             | 24.5304                      |
| 395                             | 20.451                       |  | 395                             | 24.4873                      |
| 394                             | 20.4502                      |  | 394                             | 24.4508                      |
| 393                             | 20.457                       |  | 393                             | 24.4543                      |
| 392                             | 20.4635                      |  | 392                             | 24.4766                      |
| 391                             | 20.4562                      |  | 391                             | 24.467                       |
| 390                             | 20.4748                      |  | 390                             | 24.4731                      |
| 389                             | 20.4828                      |  | 389                             | 24.4664                      |
| 388                             | 20.4921                      |  | 388                             | 24.4512                      |
| 387                             | 20.5137                      |  | 387                             | 24.485                       |
| 386                             | 20.5243                      |  | 386                             | 24.4882                      |
| 385                             | 20.537                       |  | 385                             | 24.4723                      |
| 384                             | 20.53                        |  | 384                             | 24.4777                      |
| 383                             | 20.5091                      |  | 383                             | 24.4205                      |
| 382                             | 20.4982                      |  | 382                             | 24.4331                      |
| 381                             | 20.4867                      |  | 381                             | 24.4308                      |
| 380                             | 20.4974                      |  | 380                             | 24.4413                      |
| 379                             | 20.5128                      |  | 379                             | 24.4548                      |
| 378                             | 20.5252                      |  | 378                             | 24.4329                      |
| 377                             | 20.533                       |  | 377                             | 24.4431                      |
| 376                             | 20.549                       |  | 376                             | 24.4017                      |
| 375                             | 20.5672                      |  | 375                             | 24.4495                      |
| 374                             | 20.5423                      |  | 374                             | 24.4512                      |

## FIG. 81

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 373                             | 20.5137                      |  | 373                             | 24.4121                      |
| 372                             | 20.4948                      |  | 372                             | 24.4155                      |
| 371                             | 20.4471                      |  | 371                             | 24.3647                      |
| 370                             | 20.6176                      |  | 370                             | 24.433                       |
| 369                             | 20.6285                      |  | 369                             | 24.4398                      |
| 368                             | 20.63                        |  | 368                             | 24.4208                      |
| 367                             | 20.6378                      |  | 367                             | 24.4377                      |
| 366                             | 20.6263                      |  | 366                             | 24.3924                      |
| 365                             | 20.6304                      |  | 365                             | 24.3864                      |
| 364                             | 20.5925                      |  | 364                             | 24.3719                      |
| 363                             | 20.5674                      |  | 363                             | 24.3544                      |
| 362                             | 20.5724                      |  | 362                             | 24.3364                      |
| 361                             | 20.5897                      |  | 361                             | 24.325                       |
| 360                             | 20.5923                      |  | 360                             | 24.3148                      |
| 359                             | 20.5976                      |  | 359                             | 24.3192                      |
| 358                             | 20.5941                      |  | 358                             | 24.3294                      |
| 357                             | 20.5357                      |  | 357                             | 24.3049                      |
| 356                             | 20.5327                      |  | 356                             | 24.3265                      |
| 355                             | 20.5756                      |  | 355                             | 24.3461                      |
| 354                             | 20.5876                      |  | 354                             | 24.3463                      |
| 353                             | 20.6694                      |  | 353                             | 24.3066                      |
| 352                             | 20.6807                      |  | 352                             | 24.259                       |
| 351                             | 20.6526                      |  | 351                             | 24.1875                      |
| 350                             | 20.5758                      |  | 350                             | 24.1681                      |
| 349                             | 20.5538                      |  | 349                             | 24.2042                      |
| 348                             | 20.5614                      |  | 348                             | 24.2366                      |
| 347                             | 20.5513                      |  | 347                             | 24.2744                      |
| 346                             | 20.6026                      |  | 346                             | 24.27                        |

## FIG. 82

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 345                             | 20.5842                      |  | 345                             | 24.2726                      |
| 344                             | 20.5875                      |  | 344                             | 24.2595                      |
| 343                             | 20.5753                      |  | 343                             | 24.2884                      |
| 342                             | 20.5627                      |  | 342                             | 24.3097                      |
| 341                             | 20.5936                      |  | 341                             | 24.2186                      |
| 340                             | 20.6817                      |  | 340                             | 24.4226                      |
| 339                             | 20.6141                      |  | 339                             | 24.3418                      |
| 338                             | 20.6054                      |  | 338                             | 24.2955                      |
| 337                             | 20.6289                      |  | 337                             | 24.3183                      |
| 336                             | 20.6219                      |  | 336                             | 24.2753                      |
| 335                             | 20.6507                      |  | 335                             | 24.2949                      |
| 334                             | 20.6177                      |  | 334                             | 24.2512                      |
| 333                             | 20.5812                      |  | 333                             | 24.2405                      |
| 332                             | 20.5679                      |  | 332                             | 24.2144                      |
| 331                             | 20.5333                      |  | 331                             | 24.204                       |
| 330                             | 20.547                       |  | 330                             | 24.1824                      |
| 329                             | 20.555                       |  | 329                             | 24.137                       |
| 328                             | 20.5357                      |  | 328                             | 24.1176                      |
| 327                             | 20.5497                      |  | 327                             | 24.1288                      |
| 326                             | 20.5702                      |  | 326                             | 24.1553                      |
| 325                             | 20.5403                      |  | 325                             | 24.1866                      |
| 324                             | 20.5184                      |  | 324                             | 24.1403                      |
| 323                             | 20.541                       |  | 323                             | 24.1148                      |
| 322                             | 20.5017                      |  | 322                             | 24.0971                      |
| 321                             | 20.5689                      |  | 321                             | 24.0591                      |
| 320                             | 20.5425                      |  | 320                             | 24.0259                      |
| 319                             | 20.5033                      |  | 319                             | 24.0071                      |
| 318                             | 20.4925                      |  | 318                             | 23.9693                      |

**FIG. 83**

| Tape in black                   |                              |  | Tape in white                   |                              |
|---------------------------------|------------------------------|--|---------------------------------|------------------------------|
| Wavelength<br>( $\mu\text{m}$ ) | Light transmittance<br>T (%) |  | Wavelength<br>( $\mu\text{m}$ ) | Light transmittance T<br>(%) |
| 317                             | 20.3814                      |  | 317                             | 23.9191                      |
| 316                             | 20.3944                      |  | 316                             | 23.9077                      |
| 315                             | 20.3611                      |  | 315                             | 23.8309                      |
| 314                             | 20.3148                      |  | 314                             | 23.7724                      |
| 313                             | 20.3263                      |  | 313                             | 23.7474                      |
| 312                             | 20.3185                      |  | 312                             | 23.7024                      |
| 311                             | 20.268                       |  | 311                             | 23.6667                      |
| 310                             | 20.2401                      |  | 310                             | 23.6223                      |
| 309                             | 20.2116                      |  | 309                             | 23.5775                      |
| 308                             | 20.1932                      |  | 308                             | 23.5861                      |
| 307                             | 20.2089                      |  | 307                             | 23.571                       |
| 306                             | 20.2418                      |  | 306                             | 23.5969                      |
| 305                             | 20.2418                      |  | 305                             | 23.5923                      |
| 304                             | 20.2126                      |  | 304                             | 23.5743                      |
| 303                             | 20.2326                      |  | 303                             | 23.5207                      |
| 302                             | 20.1922                      |  | 302                             | 23.4827                      |
| 301                             | 20.2358                      |  | 301                             | 23.4931                      |
| 300                             | 20.2827                      |  | 300                             | 23.4682                      |

## 1

## TAPE FOR SLIDE FASTENER

## CROSS REFERENCE TO RELATED APPLICATIONS

This application is based on Chinese Patent Application (No. 201711249063.0) filed on Dec. 1, 2017 and Chinese Utility Model Application (No. 201721651179.2) filed on Dec. 1, 2017, the contents of which are incorporated herein by way of reference.

## BACKGROUND

The present invention relates to a tape for a slide fastener.

The present invention also relates to a slide fastener comprising the above-mentioned tape for a slide fastener.

As a daily necessity, slide fasteners are widely used in various fields, especially in a large number of articles such as clothing, bags, etc. At present, there are mainly three kinds: nylon slide fasteners, resin slide fasteners and metal slide fasteners, and each has a tape, slide-fastener elements, a slider and other main components, regardless of the kind of the slide fasteners. In terms of functions, slide fasteners are mainly used to achieve opening and closing of items; however, in some industries, especially the clothing industry, slide fasteners are sometimes required to have other functions, such as light weight. In Chinese invention patent application No. 201080069345.2, the description discloses a woven tape (i.e., a tape) for a slide fastener, which, by setting yarn count of warps of the yarns forming the woven tape, weave density of the warps (i.e., yarn count density of the warps), yarn count of wefts, and weave density of the wefts (i.e., yarn count density of the wefts), provides a woven tape having both light weight and strength for a slide fastener. However, with technology development, there is a demand for lighter weight of tapes, and obviously, a tape in the prior art cannot meet the demand for lighter weight. In addition, since the length of the tape is much larger than the width thereof, when a slide fastener having the above tape is attached to an article, the tape is subjected to a large force in the width direction thereof, and due to the lightweight design of the tape, the side tensile strength is very weak, which in turn causes the tape to be extremely undurable.

## SUMMARY

In view of the aforementioned shortcomings of the prior art, an object of the present invention is to provide a tape for a slide fastener and a slider fastener, which can achieve lighter weight and effectively improve the side tensile strength of the tape simultaneously.

To achieve the above object, the present invention provides a tape for a slide fastener, wherein, for warps among yarns forming the tape, yarn count is set to 22-28 dTex and weave density is set to 205-231 yarns/inch, and for wefts among yarns forming the tape, yarn count is set to 81-87 dTex and weave density is set to 42-48 yarns/inch, and the weft is a multifilament formed by bundling 33-39 monofilaments. By setting the warp count, the weave density, the weft count and the weave density for the yarns forming the tape for a slide fastener, as well as setting the multifilament structure of the wefts, a tape with lighter weight is obtained, and the strength of the tape itself and especially the side tensile strength of the tape along the width direction thereof is effectively improved simultaneously, thereby greatly improving durability of the tape, making the tape thin,

## 2

lightweight and strong, and thus making the tape meet requirements of various aspects.

In a preferred embodiment of the above tape for a slide fastener, the yarn count of the warps is set to 25 dTex, the weave density of the warps is set to 210-226 yarns/inch, the yarn count of the wefts is set to 84 dTex, the weave density of the wefts is set to 43-46 yarns/inch, and the weft is multifilament formed by bundling 36 monofilaments.

After the tape is woven by using the features set as above, 10 the tape has a thickness of 0.1-0.2 mm, which is lighter and thinner than a tape in the prior art, thereby achieving lighter weight of the tape.

Further, when using the yarns to weave the tape, the warps and the wefts are interwoven one by one, and the thus-woven tape is a plain woven construction, which ensures strength and durability of the tape; moreover, as the warp and the weft are both very fine, the tape with a plain weave still has good flexibility, thereby ensuring the texture of the tape.

20 The tape woven by using the features set as above is very thin and light, and can have transparency even without using transparent yarns. In the embodiment, the light transmittance of the tape is 15%-30%.

25 Preferably, in order to further increase the light transmittance of the tape, the tape is made from one of polyethylene terephthalate, polypropylene, and polyamide.

In a preferred embodiment of the above tape for a slide fastener, an outer periphery of the tape has a tape edge portion. The tape edge portion is obtained by ultrasonic-wave cutting, which, under the premise of no need to provide a selvedge thread, can effectively prevent looseness of the yarns at the tape edge portion of the tape, and also ensures that the thickness of the tape edge portion is very approximate to the thickness of the rest part of the tape.

30 The present invention also provides a slide fastener comprising two rows of fastener stringers, a slider, and a pair of tapes as described above, wherein the inner-side edges of the pair of tapes is each provided with one row of the fastener stringer, and the slider is clamped on the two rows of 40 fastener stringers to achieve engagement or disengagement of the two rows of fastener stringers.

35 In a preferred embodiment of the above slide fastener, the slide fastener is a nylon slide fastener, and the fastener stringer is in a spiral-coil shape and is sewn and fixed to the tape by an element sewing thread.

In a preferred embodiment of the above nylon slide fastener, there is a folded portion formed by folding the tape along the width direction thereof at the inner-side edge of the tape. The folded portion and a portion of the tape that 50 overlaps with the folded portion form an element attaching portion of the tape. The fastener stringer is sewn and fixed to the element attaching portion by the element sewing thread. Along the width direction of the tape, the element sewing thread sewn on the element attaching portion is 55 located between both ends of the element attaching portion, to facilitate the sewing of the fastener stringers.

As described above, the tape for a slide fastener and the slide fastener according to the present invention, have the following advantages.

60 In the above-described tape for a slide fastener and the above-described slide fastener, by setting the warp count, the weave density, the weft count and the weave density for the yarns forming the tape, as well as setting the multifilament structure of the wefts, the tape with lighter weight is obtained, and the strength of the tape itself and especially the side tensile strength of the tape along the width direction thereof is effectively improved simultaneously, thereby 65

greatly improving durability of the tape, making the tape thin, lightweight and strong, and thus making the tape meet requirements of various aspects.

#### BRIEF DESCRIPTION OF DRAWINGS

FIG. 1 is a schematic structural view of a tape in the present application.

FIG. 2 is a diagram showing a corresponding relationship between light transmittance and light wavelength, when the tape in the present application is in two colors, i.e., in black and in white.

FIG. 3 is a schematic structural view of a nylon slide fastener in the present application.

FIG. 4 is a cross-sectional view of FIG. 3.

FIGS. 5 to 83 are tables showing a light transmittance of tape in black and tape in white in correspondence with irradiation of different wavelengths of light.

#### DETAILED DESCRIPTION OF EXEMPLARY EMBODIMENTS

Specific embodiments are provided to describe implementation of the present invention, and other advantages and functions of the present invention can be easily understood by a person skilled in the art from the disclosure in the following description.

It should be noted that, the structures, scales, sizes and the like shown in all the drawings, are only used to match the content disclosed in the specification, for being read and understood by a person skilled in the art, instead of limiting restricted implementation conditions of the present disclosure, and thus do not have any essential technical meaning. Any modification in structure, change in scale, or adjustment in size should fall within the scope of the technical content disclosed by the present disclosure without influencing the generated efficacy and achieved objective of the present disclosure. Meanwhile, some words such as "upper", "lower", "left", "right", "middle", and "a" quoted in the specification are only used for clarifying the illustration, instead of limiting the implementation scope of the present disclosure, and any change or adjustment of relative relationships thereof without essentially changing the technical content should be considered as falling within the scope of implementation of the present disclosure.

In the following embodiments, directions are defined as follows: a longitudinal direction of a slide fastener is defined as a front-rear direction; a width direction of the slide fastener is defined as a left-right direction; a direction orthogonal to both the front-rear direction and the left-right direction is defined as an up-down direction; further, a direction in which the slider 5 moves toward a top stop 7 of the slide fastener is the front direction, and a direction in which a slider 5 moves toward a bottom stop 8 of the slide fastener is a rear direction. Thus, the front-rear direction coincides with the moving direction of the slider 5 in the slide fastener, and the up-down direction coincides with the thickness direction of a tape 3 in the slide fastener. Alternatively, as shown in FIG. 3, an upper side of the paper surface is a front direction, a lower side of the paper surface is a rear direction, a left side of the paper surface is a left direction, a right side of the paper surface is a right direction, a front side of the paper surface is an up direction, and a back side of the paper surface is a down direction.

The present invention provides the tape 3 for a slide fastener, which achieves the lighter weight and thinness of the tape 3, and can ensure the strength of the tape 3,

especially the side tensile strength of the tape 3 along the width direction thereof. The tape 3 for a slide fastener adopts the following configuration: as shown in FIG. 1, for warps 1 (i.e., the vertical yarns extending front-to-rear) among the 5 yarns forming the tape 3, the yarn count is set to 22-28 dTex and the weave density is set to 205-231 yarns/inch (i.e., 80-91 yarns/cm); for wefts 2 (i.e., the transverse yarns extending left-to-right) among the yarns forming the tape 3, the 10 yarn count is set to 81-87 dTex and the weave density is set to 42-48 yarns/inch (i.e., 16-19 yarns/cm), and the weft 2 is a multifilament formed by bundling 33-39 monofilaments. In the tape 3 for a slide fastener, by setting the warp count, the weave density of the warp, the weft count and the weave density of the weft for the yarns forming the tape 3, 15 as well as setting the multifilament structure of the wefts, the tape 3 is made thinner and more lightweight. In particular, because the tape 3 has a relatively long length in the front-rear direction and a relatively short width in the left-right direction, so, after the slide fastener is attached to 20 an article such as clothes, forces applied to the slide fastener mainly come from the width direction of the slide fastener. In other words, the tape 3 mainly bears side tensile forces in the width direction thereof. In the present application, among the yarns forming the tape 3, the weft 2 is always 25 thicker than the warp 1, and each of the wefts 2 is set to be a multifilament formed by bundling 33-39 monofilaments, which can increase the side tensile strength of the tape 3 in the width direction thereof to a large extent, making the extremely lightweight and thin tape 3 durable. Therefore, the 30 tape 3 for a slide fastener according to the present application is thin, lightweight and strong, and thus can meet requirements of various aspects.

In a preferred embodiment of the above tape for a slide fastener, the yarn count of the warps 1 is set to 25 dTex (i.e., 35 22.5 D), the weave density of the warps 1 is set to 210-226 yarns/inch (i.e., 83-89 yarns/cm), the yarn count of the wefts 2 is set to 84 dTex, the weave density of the wefts 2 is set to 43-46 yarns/inch (i.e., 17-18 yarns/cm), the warp 1 is a monofilament, and the weft 2 is a multifilament formed by 40 bundling 36 monofilaments. In this way, under the premise of ensuring the strength of the tape 3, the lightness and thinness of the tape 3 can be maximized.

Further, when using the yarns to weave the tape 3, the warps 1 and the wefts 2 are interwoven one by one, and the 45 thus-woven tape 3 is entirely a plain woven construction, which ensures strength and durability of the tape 3 and makes the appearance of the tape 3 uniform. Moreover, as the warp 1 and the weft 2 are both very fine, even though the tape 3 is entirely a plain woven construction, the tape 3 still 50 has good flexibility, thereby ensuring the texture of the tape 3. In production of the tape 3, firstly, a tape blank woven from the warps 1 and the wefts 2 is obtained, then the tape blank is subjected to ultrasonic-wave cutting according to a required size of the tape 3, thereby obtaining the tape 3. The 55 front edge, the rear edge, the left edge and the right edge of the tape 3 are all tape edge portions 31 obtained by ultrasonic-wave cutting of the tape blank. Thus, the tape edge portions 31 are very smooth, and no fluffing, snagging, deformation, and the like phenomenon occurs at the tape edge portions 31, so that, under the premise of no need to provide a selvedge thread, the tape 3 can effectively prevent 60 looseness of the yarns at the tape edge portions 31. In addition, as the tape 3 is very lightweight and thin, the thickness of the tape 3 at the tape edge portions 31 is very 65 approximate to the thickness of the rest part of the tape 3 after the ultrasonic-wave cutting, and it is visually impossible to recognize the difference between the thickness of the

tape edge portions 31 and the thickness of the rest part of the tape 3, which greatly improves the uniformity and aesthetics of the appearance of the tape 3.

The tape 3 woven by using the features set as above has a thickness of 0.1-0.2 mm which is lighter and thinner than a tape in the prior art, thereby achieving lighter weight of the tape 3. In addition, as the tape 3 is very thin and lightweight, the tape 3 can have transparency even without using transparent yarns. A light transmittance experiment was carried out respectively on the tape 3 in black and the tape 3 in white by using a spectrophotometer, and the experimental results are shown in FIGS. 5 to 83 and FIG. 2. In FIG. 2, curve A1 is an experimental result curve for the tape 3 in black, and curve A2 is an experimental result curve for the tape 3 in white, and it can be seen that the light transmittance of the tape 3 is 15%-30%, the light transmittance of the tape 3 in black is about 20.22%, and the light transmittance of the tape 3 in white is about 24.53%.

FIGS. 5 to 83 show a light transmittance of tape in black and tape in white in correspondence with irradiation of different wavelengths of light.

To further increase the light transmittance of the tape 3, the tape 3 is made from one of polyethylene terephthalate (PET), polypropylene (PP), and polyamide (PA).

The present invention also provides a slide fastener, as shown in FIG. 3, the slide fastener mainly comprises a pair of tapes 3 as described above, two rows of fastener strings 4, a slider 5, a pull tab 6, a top stop 7 and a bottom stop 8.

The two tapes 3 in the pair of tapes 3 extend front-to-rear and are arranged side by side; the two rows of fastener strings 4 are respectively disposed on the inner-side edges of the respective tapes 3, and each row of fastener string 4 is composed of a plurality of fastener elements arranged one behind the other.

The slider 5 is clamped on the two rows of fastener strings 4 and moves back and forth along the extending direction of the fastener strings 4, for achieving engagement or disengagement of the two rows of fastener strings 4.

The pull tab 6 is mounted on the slider 5, so that a user can hold the pull tab 6 with a hand to bring the slider 5 to move back and forth; the top stop 7 is disposed at the front end of the fastener strings 4, and is used for restricting the slider 5 from being detached from the fastener strings 4 forwardly from the front end of the fastener strings 4 when the slide fastener is pulled to close.

The bottom stop 8 is disposed at the rear end of the fastener strings 4, and is used for restricting the slider 5 from being detached from the fastener strings 4 backwardly from the rear end of the fastener strings 4 when the slide fastener is pulled to open, and the bottom stop 8 also prevents the rear ends of the two rows of fastener strings 4 from being separated from each other when the two rows of fastener strings 4 are engaged.

Preferably, the slide fastener is a nylon slide fastener, in other words, a coil-type slide fastener; in the nylon slide fastener, as shown in FIG. 3 and FIG. 4, the fastener stringer 4 is in a spiral-coil shape, and is sewn and fixed to the tape 3 by an element sewing thread 9.

Further, each of the tapes 3 has an element attaching portion 32 and a tape body portion 33; the element attaching portion 32 is located on the inner side of the tape 3 and extends front-to-rear and is used for attaching of the fastener

stringer 4; except the element attaching portion 32, the rest part of the tape 3 forms the tape body portion 33; in the nylon slide fastener, the fastener stringer 4 is sewn and fixed to the element attaching portion 32 by the element sewing thread 9.

As the tape 3 is very lightweight and thin, in order to facilitate sewing of the fastener stringers 4, the element attaching portion 32 has a two-layer (i.e., upper-and-lower-layer) structure; specifically, as shown in FIG. 4, the inner-side edge of the tape 3 is formed with a folded portion 34 by folding along the width direction of the tape 3, and the folded portion 34 is located on the lower side; the folded portion 34 and a portion of the tape 3 that overlaps with the folded portion 34 together form the element attaching portion 32 of the tape 3; thus, the portion of the tape 3 that is located above the folded portion 34 and overlaps with the folded portion 34 forms the upper-layer structure of the element attaching portion 32, while the folded portion 34 forms the lower-layer structure of the element attaching portion 32; hence, the thickness and hardness of the element attaching portion 32 with the two-layer (i.e., the upper-and-lower-layer) structure are remarkably improved, thus facilitating sewing of the fastener stringers 4.

Moreover, as shown in FIG. 4, along the width direction of the tape 3, the element sewing thread 9 sewn on the element attaching portion 32 is located between both ends of the element attaching portion 32, which means that, the width of the element attaching portion 32 is larger than the distance between the two segments (i.e., left-and-right segments) of the element sewing thread 9 sewn on the element attaching portion 32, that is, the left end of the element attaching portion 32 goes leftward beyond a left segment 91 of the element sewing thread on the element attaching portion 32, and the right end of the element attaching portion 32 goes rightward beyond a right segment 92 of the element sewing thread on the element attaching portion 32.

In summary, the present invention effectively overcomes various shortcomings in the prior art, and has a high utilization value in industry.

The above-described embodiments are merely for illustration of the principle and efficacy of the present invention by way of examples, and are not intended to limit the present invention. Modifications or changes can be made to the above-described embodiments by a person skilled in the art, without departing from the spirit and scope of the present invention. Thus, all equivalent modifications or changes made by a person having common knowledge in the art, without departing from the spirit and technical ideas disclosed by the present invention, shall still be encompassed by the claims of the present invention.

What is claimed is:

1. A fastener tape for a slide fastener, wherein a yarn count of warps among yarns forming the fastener tape is set to 22-28 dTex, a weave density of the warps is set to 205-231 yarn/inch, a yarn count of wefts among the yarns forming the fastener tape is set to 81-87 dTex, a weave density of the wefts is set to 42-48 yarns/inch, the wefts are multifilaments formed by bundling 33-39 monofilaments, and a light transmittance of the fastener tape is 15%-30%.